



US007175954B2

(12) **United States Patent**  
Sakimura et al.

(10) Patent No.: US 7,175,954 B2  
(45) Date of Patent: Feb. 13, 2007

(54) ELECTROPHOTOGRAPHIC PHOTORECEPTOR

2003/0190546 A1\* 10/2003 Yoshino et al. .... 430/124

(75) Inventors: **Tomoko Sakimura**, Hino (JP); **Toyoko Shibata**, Zama (JP)

## FOREIGN PATENT DOCUMENTS

(73) Assignee: **Konica Minolta Holdings, Inc.**, Tokyo  
(JP)

JP 63-065449 3/1988  
JP 03-149560 6/1991  
JP 05-025102 2/1993

(\*) Notice: Subject to any disclaimer, the term of this patent is extended or adjusted under 35 U.S.C. 154(b) by 387 days.

\* cited by examiner

(21) Appl. No.: 10/805,962

*Primary Examiner*—Mark A. Chapman

(22) Filed: Mar. 22, 2004

(74) Attorney, Agent, or Firm—Lucas & Mercanti, LLP

(65) **Prior Publication Data**

US 2004/0191654 A1 Sep 30, 2004

(30) Foreign Application Priority Data

|               |      |       |             |
|---------------|------|-------|-------------|
| Mar. 31, 2003 | (JP) | ..... | 2003-093896 |
| Mar. 31, 2003 | (JP) | ..... | 2003-093897 |
| May 22, 2003  | (JP) | ..... | 2003-144707 |
| Aug. 28, 2003 | (JP) | ..... | 2003-304318 |

An electrophotographic photoreceptor comprising a support and a photosensitive layer is disclosed. The photosensitive layer contains a mixture of compounds represented by Formula (1) having different n and  $(R_p+R_s)$  is not more than 99%, wherein  $R_p$  is a ratio of a component having the maximum content in the mixture and  $R_s$  is a ratio of a component having the content next to the maximum content in percent.

(51) **Int. Cl.**  
**G03G 15/02** (2006.01)

$$X-(CTM\text{-group})_n-Y \quad (1)$$

(52) U.S. Cl. .... 430/58.05; 430/58.85;  
430/78; 430/56

In the formula, CTM-group is a charge transfer group; X and Y are each a hydrogen atom, a halogen atom or a monovalent organic group; and n is an integer of from 0 to 10, provided that n is an integer of from 1 to 10 when both X and Y are hydrogen atom or a halogen atom. A processing cartridge comprising the electrophotographic photoreceptor is also disclosed.

(56) **References Cited**

## U.S. PATENT DOCUMENTS

5,427,879 A \* 6/1995 Takano et al. .... 430/58.45

17 Claims, 1 Drawing Sheet



FIG. 1



## 1

ELECTROPHOTOGRAPHIC  
PHOTORECEPTOR

## FIELD OF THE INVENTION

The present invention relates to an electrophotographic photoreceptor, a processing cartridge, an image forming apparatus and an image forming method to be used for image formation by the electrophotographic process, further in detail, relates to the electrophotographic photoreceptor, processing cartridge, image forming apparatus and image forming method to be used for image formation by the electrophotographic process commonly used in the field of copying machine and printer.

## BACKGROUND OF THE INVENTION

Recently, organic photoreceptor has become the principal type of electrophotographic photoreceptors in place of an inorganic photoreceptor. The reason being that organic photoreceptor has a wider selection range of a photosensitive material, superiority in environmental suitability and lower cost compared with an inorganic photoreceptor such as a selenium photoreceptor and an amorphous silicon photoreceptor.

Besides, digital image forming system using a LED or a laser as the light source is rapidly permeating in the field of a printer for personal computer and usual copying machine for reason of ease of image processing and development of a combined machine function. In addition, technique has been developed to progress the precision of the image and to form a high quality electrophotographic image. For example, technique is disclosed in which imagewise exposure is carried out by a laser beam having small spotting area for raising the dot density to form a high precision latent image, and the latent image is developed by a fine particle toner, c.f. Publication 1.

An organic photoreceptor is required for forming such the high quality image, which has high sensitivity and stable properties concerning the thermal environment.

Hitherto, for satisfying such the requirements of organic photoreceptor, the organic photoreceptor are constituted of a photosensitive layer in which the functions are separated by a charge generation layer and a charge transfer layer, and the charge transfer layer contains a large amount of a lower molecular weight charge transfer material having a molecular weight of approximately 500. However, in the charge transfer layer having such a constitution, the quality of the layer is easily degraded and the surface of the charge transfer layer is also easily contaminated by foreign matter. The surface of the photoreceptor tends to be contaminated by paper powder or toner components during the developing process, transferring unit and cleaning unit arranged around the photoreceptor. As a result of that, recurring image defects such as a black spotting (spots in a strawberry shape) and lacking of toner transfer tends to occur. Satisfactory sensitivity is difficult to obtain in a high speed copying machine in which the duration between the exposing process and the developing process is very short or under a low temperature and/or low humidity condition. As a result of that, dot image cannot be exactly reproduced and a fine line image tends to be easily degraded.

As a measure for solving such the problem, a method using a charge transfer material having high molecular weight is developed. For example, an organic photoreceptor has been reported in Publication 2, in which a charge transfer material having a bi-styryl structure with a molecular weight

## 2

of 1,000 or more is used. Such a compound, however, cannot be uniformly dispersed in the binder resin when the compound is contained in the charge transfer layer since the compatibility of the compound with the binder resin tends to be insufficient. Consequently, the sensitivity becomes insufficient and damage such as cracking of the charge transfer layer tends to occur. Furthermore, a photoreceptor using a charge transfer material having a molecular weight of from 3,000 to 5,000 is reported in Publications 3 and 4. However, the residual potential tends to be raised on the photoreceptor using such the compound since the terminal of the compound is not blocked and the problem of the compatibility with the binder resin has not been sufficiently dissolved.

A photoreceptor is proposed in Publication 5, in the surface layer of which fluororesin particles are contained for preventing the contamination of the surface. However the use of the fluororesin particles in the surface layer tends to cause the image spreading. The mechanical strength of the surface layer also tends to be degraded and the surface of the photoreceptor is easily worn by the friction of the cleaning unit. Accordingly, a satisfactory image cannot be constantly provided.

Publication 1: Japanese Patent Publication Open to Public Inspection hereinafter referred to as JP O.P.I. Publication, No. 2001-255685.

Publication 2: JP O.P.I. Publication No. 3-149560

Publication 3: JP O.P.I. Publication No. 3-149560

Publication 4: JP O.P.I. Publication No. 5-25102

Publication 5: JP O.P.I. Publication No. 63-65449

## SUMMARY OF THE INVENTION

This invention is proposed to dissolve the foregoing problems. The objective of the invention is to prevent the defects of the image caused by the decrease of the sensitivity, which tends to occur in the course of high speed copying or copying under a low temperature and low humidity condition, by the lowering of the sharpness of the image accompanying the decreasing of image density and thinning of character image caused by the charge fluctuation of the solid black image area. Further objectives of the invention is to provide an electrophotographic photoreceptor, and a processing cartridge, an image forming method and an image forming apparatus each using the photoreceptor, by which recurring image defects such as the black spotting and the lacking of toner transfer caused by the contamination on the photoreceptor surface and the damage such as cracking of the photoreceptor surface are prevented and a clear electrophotographic image of high optical density and high resolution is continuously obtained.

As a result of the detailed investigation by the inventors on the binder resin and the charge transfer material constituting the charge transfer layer, it was discovered that as the compatibility of the charge transfer material with the binder resin is raised, the high speed response of the sensitivity under low temperature and low humidity is improved, the contamination of the surface of the photoreceptor is inhibited to prevent the occurrence of the recurring image defects such as black spotting and the lack of toner transfer, damage such as the cracking, and a clear image of high density and high resolution can be stably obtained when a mixture of compounds each having different molecular weight from each other is used as the charge transfer material.

The invention is described below.

1. An electrophotographic photoreceptor comprising a support and a photosensitive layer, wherein the photosensitive layer contains a mixture of two or more compounds

each of which is represented by Formula (1) having a specific number  $n$  different each other,



wherein CTM-group is a charge transfer group; X and Y are each a hydrogen atom, a halogen atom or a mono-valent organic group; and n is an integer of 0 to 10, provided that n is not 0 when both X and Y are a hydrogen atom or a halogen atom, and

(Rp+Rs) is not more than 99%,

wherein  $R_p$  is a content of a compound represented by Formula (1) which has a first specific number  $n$  and a maximum content in the mixture, and  $R_s$  is a content of a component represented by Formula (1) which has a second specific number  $n$  and a content next to the maximum content based on weight in percent.

2. An electrophotographic photoreceptor comprising an electroconductive substrate having thereon a charge generation layer containing a charge transfer material and a charge transfer layer containing a charge generation material, wherein the charge transfer material is a mixture of compounds as specified in item 1 above.

3. The electrophotographic photoreceptor described in 1 or 2, wherein  $(Rp+Rs)$  is from 30% to 99%.

4. The electrophotographic photoreceptor described in any one of 1 through 3, wherein the weight average molecular weight is from 650 to 2,500.

5. The electrophotographic photoreceptor described in 4, wherein the weight average molecular weight is from 800 to 2,000.

6. The electrophotographic photoreceptor described in any one of 3 through 5, wherein  $(Rp+Rs)$  is from 45% to 90%.

7. The electrophotographic photoreceptor described in any one of 1 through 6, wherein the CTM-group, X and Y in Formula (1) are each represented by following formula A, respectively.

### Formula A:



In Formula A,  $Ar_1$  is a substituted or unsubstituted mono-valent aromatic group;  $Ar_2$  is a di-valent substituted or unsubstituted aromatic group, a di-valent furan or thiophene group; or a group represented by Formula (2);  $R_1$  through  $R_3$  are each a hydrogen atom, a substituted or unsubstituted alkyl group or a substituted or unsubstituted mono-valent aromatic group; A is a di-valent group having a triarylamino group or a group represented by the following Formula (3). Each of the plural  $Ar_1$ ,  $R_1$ ,  $R_2$  and  $R_3$  may be the same with or different from each other, and p and q are each an integer of 0 or 1.



Formula (2)

In the above, Z is a single bond, an oxygen atom, a sulfur atom, a  $-\text{CH}=\text{CH}-$  group or a  $-\text{C}(\text{R}_4)(\text{R}_5)-$  group, and  $\text{R}_4$  and  $\text{R}_5$  may be bonded together.



Formula (3)

In the above,  $Z_1$  is a single bond, an alkylene group, an oxygen atom or a sulfur atom; and  $R_6$  is a substituted or unsubstituted alkyl group, or substituted or unsubstituted aromatic group.

- 25 8. The electrophotographic photoreceptor described in any one of 1 through 6, wherein CTM-group, X and Y in Formula (1) have each the chemical structures represented by the following Formula B, respectively.

### Formula B:



45 In the above,  $Ar_2$  is a substituted or unsubstituted di-  
aromatic group, a di-  
50 valent furan or thiophene group or a  
group represented by Formula (2);  $R_1$  through  $R_3$  are each a  
hydrogen atom, a substituted or unsubstituted alkyl group, or  
a substituted or unsubstituted mono-  
valent aromatic group;  
A is a divalent group having a triarylmino group or a group  
represented by Formula (3); and  $Ar_1$  is a substituted or  
unsubstituted mono-  
55 valent aromatic group; plural  $Ar_1$ ,  $R_1$ ,  
 $R_2$  and  $R_3$  each may be the same or different from each other  
and m is an integer of 0 or 1.

9. The electrophotographic photoreceptor described in any one of 7 through 8, wherein the divalent group having the triarylamino group represented by Formula A is a group represented by the following Formula (4).



Formula (4)

In the above,  $Ar_3$  is a substituted or unsubstituted mono-valent aromatic group.

10. The electrophotographic photoreceptor described in 9, wherein the group represented by  $Ar_3$  is a group represented by Formula (5)



Formula (5)

In the above,  $R_{31}$ ,  $R_{32}$ ,  $R_{33}$ ,  $R_{34}$  and  $R_{35}$  are each a hydrogen atom or an alkyl group having from 1 to 4 carbon atoms and at least one of  $R_{31}$  and  $R_{35}$  is an alkyl group having from 1 to 4 carbon atoms.

11. The electrophotographic photoreceptor described in any one of 7 through 8, wherein the di-valent group having a triarylarnino group represented by Formula A is a group represented by Formula (6).



Formula (6)

In Formula (6),  $X_2$  is a single bond, a substituted or unsubstituted alkylene group, or a substituted or unsubstituted di-valent aromatic group;  $Ar_4$  and  $Ar_5$  are each a substituted or unsubstituted mono-valent aromatic group.

12. The electrophotographic photoreceptor described in 8, wherein  $Ar_1$  is a group represented by Formula (7).



Formula (7)

In Formula (7),  $R_{41}$ ,  $R_{42}$ ,  $R_{43}$ ,  $R_{44}$ ,  $R_{45}$ ,  $R_{51}$ ,  $R_{52}$ ,  $R_{53}$ ,  $R_{54}$  and  $R_{55}$  are each a hydrogen atom or an alkyl group having from 1 to 4 carbon atoms, provided that at least one of  $R_{41}$ ,  $R_{45}$ ,  $R_{51}$  and  $R_{55}$  is an alkyl group having from 1 to 4 carbon atoms.

13. The electrophotographic photoreceptor described in any one of 1 through 6, wherein the CTM-group in Formula (1), X, and Y are each represented by Formula C.



Formula C

10 In Formula C,  $Ar_1$  is a substituted or unsubstituted mono-valent aromatic group;  $Ar_6$  is a substituted or unsubstituted di-valent aromatic group, or a group represented by the following Formula (8); R is a substituted or unsubstituted alkyl group or a substituted or unsubstituted mono-valent aromatic group. Plural  $Ar_1$ ,  $Ar_6$  and R may be the same as or different from each other.



Formula (8)

In Formula (8),  $Z_3$  is an oxygen atom, a sulfur atom, a  $-\text{CH}=\text{CH}-$  group or a  $-\text{CH}_2-\text{CH}_2-$  group; and  $R_{81}$  and  $R_{82}$  are each a hydrogen atom or an alkyl group having from 1 to 4 carbon atoms.

14. A processing cartridge which includes as a unit the electrophotographic photoreceptor described in the foregoing 1, and at least one of a charging unit for uniformly charging the surface of the electrophotographic photoreceptor, a latent image forming unit for forming a latent image on the charged electrophotographic photoreceptor, a developing unit for visualizing the latent image formed on the electrophotographic photoreceptor, a transferring unit for transferring the toner image visualized on the electrophotographic photoreceptor to a recording material, a discharging unit for removing the charge on the electrophotographic photoreceptor and a cleaning unit for removing the toner remaining on the electrophotographic photoreceptor, and is installed and released to from the main body of the image forming apparatus as necessary.

#### BRIEF DESCRIPTION OF THE DRAWING

FIG. 1 shows the cross section of the constitution of an image forming apparatus as an example of the image forming method according to the invention.

#### DETAILED DESCRIPTION OF THE INVENTION

55 The present invention will be described in detail below. The image defects caused by insufficiency of high speed response of photosensitivity which tends to occur in image formation at high speed and under a low temperature and low humidity conditions and various other kinds of defects which tend to occur under high temperature and high humidity condition are prevented to provide an electrophotographic image with high image density and high sharpness by the use of the electrophotographic photoreceptor, processing cartridge, image forming method and image forming apparatus of this invention.

The electrophotographic photoreceptor of the invention contains a mixture of compounds represented by Formula

(1) in which  $n$  has a range of distribution and  $(Rp+Rs)$  is not more than 99% when  $Rp$  represents the ratio of a component having the maximum content in the mixture and  $Rs$  represents the ratio of a component having the content next to the maximum content.



In Formula (1), the CTM-group is a charge transfer group; X and Y are each a hydrogen atom, a halogen atom or a mono-valent organic group; and n is an integer of from 0 to 10, provided that n is an integer of from 1 to 10 when both of X and Y are hydrogen atom or a halogen atom. In such a case, it may be that either X or Y is a hydrogen atom and the other is a halogen atom.

The electrophotographic photoreceptor of the invention comprises an electroconductive substrate having thereon a charge generation layer and a charge transfer layer containing a charge transfer material in which the charge transfer material is a mixture of compounds represented by Formula (1) in which n has a range of distribution and  $(Rp+Rs)$  is not more than 99% when Rp represents the ratio of a component having the maximum content in the mixture and Rs represents the ratio of a component having the content next to the maximum content.

"The mixture of compounds represented by Formula (1) in which  $n$  has a range of distribution and  $(R_p+R_s)$  is not more than 99% when  $R_p$  represents the ratio of a component having the maximum content in the mixture and  $R_s$  represents the ratio of a component having the content next to the maximum content" means that in the mixture of compounds, compounds each of which is represented by Formula (1) and the number of the chain structure of the CTM-group or the charge transfer group differ from each other, are in a mixed state, and the sum of  $R_p$  and  $R_s$  is not more than 99% where  $R_p$  is the content of the compound having the largest presence ratio and  $R_s$  is the content of the compound having the secondary presence ratio. Therefore, the mixture of compounds contains at least three kinds of the compounds each represented by Formula (1). By the use of such a mixture of compounds, the charge transferring ability is considerably improved; the problems of lowered sensitivity caused by processing at high speed or under conditions of low temperature and low humidity can be resolved; the permeability of the solvent or the binder resin is remarkably improved; the occurrence of the black spotting and the recurring image defects such as lack of toner transfer are prevented; and in addition the damage such as cracking can be inhibited; so that the electrophotographic photoreceptor capable of forming a consistently clear electrophotographic image of high image density and high resolution can be realized.

The CTM-group in Formula (1) is a group having drift mobility of electrons or positive holes. In other word, the CTM-group is a group from which electric current caused the charge transfer can be detected by the Time-Of-Flight method.

When the CTM-group cannot exist solely itself, the CTM-group may be included within the definition of the CTM-group if a compound of the CTM-group having a hydrogen atom at the both ends thereof, and represented by  $H(\text{CTM-group})H$  has charge transferring ability.

The mixture of compounds is represented by the following Formulas A, B and C, such the mixture of compounds can be prepared by the later-mentioned synthesizing examples.



Ar<sub>1</sub> is a substituted or unsubstituted mono-valent aromatic group; Ar<sub>2</sub> is a substituted or unsubstituted di-valent aromatic group, a di-valent furan or thiophene group, or a group represented by Formula (2); R<sub>1</sub> through R<sub>5</sub> are each a hydrogen atom, a substituted or unsubstituted alkyl group or a substituted or unsubstituted mono-valent aromatic group; A is a di-valent group having a triaryl amino group or a group represented by the following Formula (3). Each of the plural Ar<sub>1</sub>, R<sub>1</sub>, R<sub>2</sub> and R<sub>3</sub> may be the same or differing from each other, and p and q are each an integer of 0 or 1.



In the above, Y is a single bond, an oxygen atom, a sulfur atom, a  $-\text{CH}=\text{CH}-$  group or a  $-\text{C}(\text{R}_4)(\text{R}_5)-$  group, and  $\text{R}_4$  and  $\text{R}_5$  may be bonded with together.



50 In the above,  $Z_1$  is a single bond, an alkylene group, an oxygen atom or a sulfur atom; and  $R_6$  is a substituted or unsubstituted alkyl group, or substituted or unsubstituted aromatic group.





Ar<sub>2</sub> is a substituted or unsubstituted di-valent aromatic group, a di-valent furan or thiophene group or a group represented by Formula (2); R<sub>1</sub> through R<sub>3</sub> are each a hydrogen atom, a substituted or unsubstituted alkyl group or a substituted or unsubstituted mono-valent aromatic group; A is a divalent group having a triaryl amino group or a group represented by Formula (3); and Ar<sub>1</sub> is a substituted or unsubstituted mono-valent aromatic group; plural B, R<sub>1</sub>, R<sub>2</sub> and R<sub>3</sub> each may be the same as or different from each other and m is an integer of 0 or 1.

In formulas A and B, the di-valent group having a triaryl amino group is a group having two bonding hands as a whole in which three bonding hands of the nitrogen atom each bonds with an aromatic ring.

In Formulas A and B, as the substituted or unsubstituted mono-valent group represented by Ar<sub>1</sub>, a substituted or unsubstituted phenyl group and a substituted or unsubstituted naphthyl group are preferable; and the substituent of these groups is preferably an alkyl group having from 1 to 4 carbon atoms, an alkoxy group, a phenyl group and a halogen atom. As the substituted or unsubstituted di-valent group represented by Ar<sub>2</sub>, a phenylene group, a naphthylene group and a biphenylene group are preferable; and a substituent of these groups is preferably an alkyl group. A di-valent furan group and a di-valent thiophene group are also preferred.

R<sub>1</sub>, R<sub>2</sub>, and R<sub>3</sub> are each preferably a hydrogen atom, a halogen atom, a substituted or unsubstituted alkyl group, a substituted or unsubstituted alkoxy group or a substituted or unsubstituted aromatic group, and are preferably a hydrogen

atom, an alkyl group and an alkoxy group each having from 1 to 4 carbon atoms, a substituted or unsubstituted phenyl group or a phenyl group having a halogen atom or an alkyl group having from 1 to 4 carbon atoms.

The di-valent group represented by A is preferably a di-valent group having a triaryl amino group represented by Formula (4) or Formula (6), in addition to the group represented by Formula (3).

A<sub>6</sub> is a substituted or unsubstituted alkyl group or a substituted or unsubstituted aromatic group, and is preferably an alkyl group having from 1 to 4 carbon atoms or a phenyl group.

Ar<sub>3</sub> is a substituted or unsubstituted mono-valent aromatic group, and preferably an unsubstituted phenyl group or a phenyl group substituted with an alkyl group having from 1 to 4 carbon atoms or an alkoxy group.

Ar<sub>4</sub> and Ar<sub>5</sub> are each a substituted or unsubstituted mono-valent aromatic group, and preferably an unsubstituted phenyl group or a phenyl group substituted with an alkyl group having from 1 to 4 carbon atoms or an alkoxy group.

Typical chemical structures of the group represented by Formulas A and B are shown below. In the invention, the mixture of the compounds or mixture of compounds each represented by the following structure and different from each other in the value of n are used as the charge transfer material. The compounds in which p or q in Formula A or m in Formula B differing from each other are different compounds even if the chemical structure of them is the same. For example, one having a value of p or q as 0 and one having the value of p or q as 1 are different compounds even when each of the compounds has following structure 1A. In addition, the compound differing in the distribution of n are different compounds even when the p or q is the same.

Specific examples of the compound represented by Formula A.

Chemical structure

No.

A

Ar<sub>1</sub>

R<sub>1</sub>

1A



H

2A



H

-continued

3A



H

4A



5A



6A



7A



8A



H

-continued

9A



H

10A



H

11A



12A



13A



14A



H

-continued

15A



H

16A



H

17A



H

18A



19A



20A



-continued

21A



22A



23A



24A



25A



26A



-continued

27A



28A



29A



30A



H

31A



H

32A



33A



-continued



-continued

41A



42A



| Chemical structure No. | Ar <sub>2</sub> | R <sub>2</sub> | R <sub>3</sub> |
|------------------------|-----------------|----------------|----------------|
| 1A                     |                 | H              | H              |
| 2A                     |                 | H              | H              |
| 3A                     |                 | H              |                |
| 4A                     |                 | H              | H              |
| 5A                     |                 | H              | H              |
| 6A                     |                 | H              | H              |
| 7A                     |                 | H              | H              |
| 8A                     |                 | H              | H              |

-continued

|     |                                                                                     |   |                                                                                       |
|-----|-------------------------------------------------------------------------------------|---|---------------------------------------------------------------------------------------|
| 9A  |    | H | H                                                                                     |
| 10A |    | H |    |
| 11A |    | H | H                                                                                     |
| 12A |    | H | H                                                                                     |
| 13A |    | H | H                                                                                     |
| 14A |   | H | H                                                                                     |
| 15A |  | H | H                                                                                     |
| 16A |  | H | H                                                                                     |
| 17A |  | H | H                                                                                     |
| 18A |  | H | H                                                                                     |
| 19A |  | H | H                                                                                     |
| 20A |  | H | H                                                                                     |
| 21A |  | H | H                                                                                     |
| 22A |  | H | H                                                                                     |
| 23A |  | H |  |

-continued

|     |  |   |   |
|-----|--|---|---|
| 24A |  | H | H |
| 25A |  | H | H |
| 26A |  | H | H |
| 27A |  | H |   |
| 28A |  | H | H |
| 29A |  | H | H |
| 30A |  | H | H |
| 31A |  | H | H |
| 32A |  | H | H |
| 33A |  | H | H |
| 34A |  | H | H |
| 35A |  | H | H |

-continued

36A



H

H

37A

CH<sub>3</sub>—

H

38A



H

39A



H

40A



H

H

41A



H

H

42A



H

H

In the above exemplified compounds, Ar<sub>1</sub>, R<sub>1</sub>, R<sub>2</sub>, and R<sub>3</sub> of Formula A are each the same, respectively. However, the invention includes a compound having different Ar<sub>1</sub>, R<sub>1</sub>, R<sub>2</sub>, and R<sub>3</sub> such that compounds represented by Formula A' are included in an example of the chemical structure of Formula (1).

In the formulas, A', Ar<sub>1</sub> and Ar<sub>1</sub>' are each a substituted or unsubstituted mono-valent aromatic group; Ar<sub>2</sub> is a substituted or unsubstituted di-valent aromatic group or a group represented by Formula (2); R<sub>1</sub>, R<sub>2</sub> and R<sub>3</sub>, and R<sub>1</sub>', R<sub>2</sub>' and R<sub>3</sub>' are each a hydrogen atom, a substituted or unsubstituted alkyl group, or a substituted or unsubstituted mono-valent aromatic group; and A is a divalent group having a triarylamino group or a group represented by Formula (3). Ar<sub>1</sub> and R<sub>1</sub>, and Ar<sub>1</sub>' and R<sub>1</sub>', may each be bonded to form a ring. P and q are each an integer of 0 or 1.



Chemical structures of typical compounds represented by Formula A' are shown below. The mixture of compounds represented by the above chemical structure is used as the charge transfer material, in which n has a range of distribution and (Rp+Rs) is not more than 99% when Rp represents the ratio of a component having the maximum content in the mixture and Rs represents the ratio of a component having the content next to the maximum content.

| Chemical structure No. | A                | Ar <sub>1</sub> | R <sub>1</sub>                                 | Ar <sub>1</sub> ' |
|------------------------|------------------|-----------------|------------------------------------------------|-------------------|
| 43A                    |                  |                 |                                                |                   |
| 44A                    |                  |                 |                                                |                   |
| Chemical structure No. | R <sub>1</sub> ' | Ar <sub>2</sub> | R <sub>2</sub> R <sub>2</sub> ' R <sub>3</sub> | R <sub>3</sub> '  |
| 43A                    |                  |                 | H H H                                          | H                 |
|                        |                  |                 |                                                |                   |
| 44A                    |                  |                 | H H H                                          |                   |
|                        |                  |                 |                                                |                   |

Synthesizing Examples of the compounds represented by Formula A are described below.

In the following synthesizing example, the raw materials are described by attaching the number shown in the scheme of the synthesis of the compound.

#### SYNTHESIZING EXAMPLE 1

50

Synthesizing of Compound 21A (p=q=0)



-continued



Placed into a 100 ml four-mouth flask equipped with a nitrogen gas inlet pipe, a cooler, a thermometer and a stirrer, were 1.68 g (0.015 moles) of potassium tert-butoxide 4 and 20 ml of tetrahydrofuran, hereinafter referred to as THF, were charged and stirred while introducing nitrogen gas.

A solution was prepared by dissolving 2.06 g (0.006 moles) of Compound 1, and 1.13 g (0.003 moles) of Compound 2 and 1.92 g (0.0063 moles) of Compound 3 dissolved in 20 ml of THF. The solution was gradually dripped into the mixture of potassium tert-butoxide 4 and THF while the temperature was maintained at 45° C. After the dripping, reaction was allowed over 5 hours while maintaining a temperature of from 45 to 50° C.

Into another 200 ml beaker, equipped with a stirrer, 20 ml of methanol was placed and stirred. The reaction liquid after a reaction of 5 hours was poured to the methanol, and 20 ml of water was further added and stirred for 30 minutes, afterwhich the liquid was subjected to filtration. The filtered precipitation was washed with about 40 ml of a mixture of methanol and water at a ratio of 1:1 and dried overnight at a temperature of from 50 to 60° C., whereby unpurified crystals were obtained.

The unpurified crystals were dissolved in 30 ml of toluene, and 3 g of Wakogel B-0, produced by Wako Pure Chemical Industries, Ltd., was added to the solution and stirred for 30 minutes and then filtered. The Wakogel B-0 was washed with 30 ml of toluene. The filtrate and the washing toluene was concentrated and dried. The dried substance was dissolved by adding 10 ml of ethyl acetate, afterwhich solution was dripped into 60 ml of methanol for

purifying by re-precipitation. By filtering and drying, 2.54 g of a compound having the chemical structure 21A ( $p=0$ ) was obtained. As a result of analysis via high speed liquid chromatography and mass spectrography, the above-obtained compound was confirmed to be a mixture of compounds having an  $n$  of from 0 to 4. The content ratio, that is, area of high speed liquid chromatograph, was  $n=0/1/2/3/4=25.4/48.8/18.1/6.3/1.4$ .

The conditions of the high speed liquid chromatography were as follows.

Measuring apparatus: Shimadzu LC6A, manufactured by Shimadzu Seisakusho Co., Ltd.

Column: CLC-ODS, manufactured by Shimadzu Seisakusho Co., Ltd.

Wavelength of detecting light: 290 nm

Moving phase: A mixture solvent of methanol and tetrahydrofuran at a ratio of 3:1.

Flowing velocity of moving phase: About 1 m/min.

The content ratio of the mixture of compounds of the invention is determined by the ratio of the area of each of the components in percent when the total content ratio was 100% after the separation by the high speed liquid chromatography. Regarding the above determining conditions, the measuring apparatus, column and moving phase may be changed as long as the components of the mixture of compounds can be clearly separated and the results the same as the invention can be obtained.

## SYNTHESIZING EXAMPLE 2

Synthesis of Compound 21A (p=1, and q=0)



Into a 100 ml four-mouth flask equipped with a nitrogen gas inlet pipe, a cooler, a thermometer and a stirrer, 1.68 g (0.015 moles) of potassium tert-butoxide 4 and 20 ml of tetrahydrofuran, hereinafter referred to as THF, were charged and stirred while introducing nitrogen gas.

A solution was prepared by dissolving 2.06 g (0.006 moles) of Compound 1 and 1.13 g (0.003 moles) of Compound 2 and 2.08 g (0.0063 moles) of Compound 3 dissolved in 20 ml of THF. The solution was gradually dripped into the mixture of potassium tert-butoxide 4 and THF while the temperature was maintained at 45° C. After the finish of the dripping, reaction was allowed over 5 hours while maintaining a temperature of from 45 to 50° C.

To another 200 ml beaker, a stirrer was equipped and 20 ml of methanol was charged and stirred. The reaction liquid after the reaction over 5 hours was poured to the methanol, and 20 ml of water was further added and stirred for 30 minutes. Thereafter the liquid was subjected to filtration. The filtered precipitation was washed by about 40 ml of a

50 mixture of methanol and water at a ratio of 1:1 and dried for one night at a temperature of from 50 to 60° C. Thus unpurified crystals were obtained.

55 The unpurified crystals were dissolved in 30 ml of toluene, and 3 g of Wakogel B-0, produced by Wako Pure Chemical Industries, Ltd., was added to the solution and stirred for 30 minutes and filtered. The Wakogel B-0 was washed by 30 ml of toluene. The filtrate and the washing toluene was concentrated and dried. The dried substance was dissolved by adding 10 ml of ethyl acetate. The solution was dripped into 60 ml of methanol for purifying by re-precipitation. By filtering and drying, 2.75 g of a compound having the chemical structure 21A (p=1 and q=0) was obtained. As a result of analysis by high speed liquid chromatography and mass spectrography, the above-obtained compound is a mixture of compounds having an n of from 0 to 4. The content ratio or area of high speed liquid chromatograph was n=0/1/2/3/4=33.4/46.8/15.0/4.0/0.8.

## Synthesis of Compound 14A (p=1 and q=0)



Into a 100 ml four-mouth flask to which a nitrogen gas inlet pipe, a cooler, a thermometer and a stirrer were equipped, 1.68 g (0.015 moles) of 4(potassium-tert-butoxide) and 20 ml of tetrahydrofuran, hereinafter referred to as THF, were charged and stirred while introducing nitrogen gas.

A solution was prepared by dissolving 1.89 g (0.006 moles) of Compound 1 and 1.13 g (0.003 moles) of Compound 2 and 1.60 g (0.0063 moles) of Compound 3 dissolved in 20 ml of THF. The solution was gradually dripped into the mixture of 4(potassium-tert-butoxide) and THF while the temperature was maintained at 45° C. After the finish of the dripping, reaction was allowed over 5 hours while maintaining a temperature of from 45 to 50° C.

To another 200 ml beaker, a stirrer was equipped and 20 ml of methanol was charged and stirred. The reaction liquid after the reaction for 5 hours was poured to the methanol, and 20 ml of water was further added and stirred for 30 minutes. Thereafter the liquid was subjected to filtration. The filtered precipitation was washed by about 40 ml of a

30 mixture of methanol and water at a ratio of 1:1 and dried for one night at a temperature of from 50 to 60° C. Thus unpurified crystals were obtained.

35 The unpurified crystals were dissolved in 30 ml of toluene, and 3 g of Wakogel B-0, produced by Wako Pure Chemical Industries, Ltd., was added to the solution and stirred for 30 minutes and filtered. The Wakogel B-0 was washed by 30 ml of toluene. The filtrate and the washing toluene was concentrated and dried. The dried substance was 40 dissolved by adding 10 ml of ethyl acetate. The solution was dripped into 60 ml of methanol for purifying by re-precipitation. By filtering and drying, 2.32 g of a compound having the chemical structure 14A (p=1 and q=0) was obtained. As a result of analysis by high speed liquid chromatography and 45 mass spectrography, the above-obtained compound is a mixture of compounds having an n of from 0 to 4. The content ratio or area of high speed liquid chromatograph was n=0/1/2/3/4=30.1/45.4/16.7/6.0/1.8.

Specific examples of Formula B



-continued

2B



3B



4B



5B



6B



7B



-continued

8B



9B



10B



11B



12B



13B



-continued

14B



15B



16B



17B



18B



19B



-continued

20B



21B



22B



23B



24B



25B



26B



-continued

27B



28B



29B



30B



| Chemical structure No. | Ar <sub>2</sub> | R <sub>1</sub> | R <sub>2</sub> | R <sub>3</sub> |
|------------------------|-----------------|----------------|----------------|----------------|
| 1B                     |                 | H              | H              | H              |
| 2B                     |                 | H              | H              | H              |
| 3B                     |                 | H              | H              | H              |
| 4B                     |                 | H              |                | H              |
| 5B                     |                 | H              | H              | H              |

-continued

|     |  |   |   |   |
|-----|--|---|---|---|
| 6B  |  | H | H | H |
| 7B  |  | H | H | H |
| 8B  |  | H |   | H |
| 9B  |  | H | H | H |
| 10B |  | H | H | H |
| 11B |  | H | H | H |
| 12B |  | H | H | H |
| 13B |  | H | H | H |
| 14B |  | H | H | H |
| 15B |  | H | H | H |
| 16B |  | H | H | H |
| 17B |  | H | H | H |
| 18B |  | H | H | H |
| 19B |  | H | H | H |

-continued

|     |  |   |   |                   |
|-----|--|---|---|-------------------|
| 20B |  | H | H | H                 |
| 21B |  | H | H | H                 |
| 22B |  | H | H | H                 |
| 23B |  | H | H | H                 |
| 24B |  | H | H | CH <sub>3</sub> — |
| 25B |  | H | H | H                 |
| 26B |  | H | H | H                 |
| 27B |  | H | H | H                 |
| 28B |  | H | H | H                 |
| 29B |  | H | H | H                 |
| 30B |  | H | H | H                 |

The above-described exemplified compounds are examples of the compound in which plural B, R<sub>1</sub>, R<sub>2</sub> and R<sub>3</sub> in Formula B are each the same. However, compounds in which plural B, R<sub>1</sub>, R<sub>2</sub> and R<sub>3</sub> are each different from the other are included in the invention. For example, the following compounds represented by Formula B' are also included in the invention as the compound represented by Formula B.

### Formula B'

### CTM-group



-continued



In Formula B',  $\text{Ar}_2$  is a substituted or unsubstituted divalent aromatic group, a furan group or a thiophene;  $\text{R}_1$ ,  $\text{R}_2$  and  $\text{R}_3$ , and  $\text{R}_1'$ ,  $\text{R}_2'$  and  $\text{R}_3'$  are each a hydrogen atom, a substituted or unsubstituted alkyl group and a substituted or unsubstituted mono-valent aromatic group; and A is a divalent group having a trarylmino group or a group represented by Formula (3).  $\text{Ar}_1$  and  $\text{Ar}_1'$  are each a substituted or unsubstituted aromatic group. m is each an integer of 0 or 1.



31B



32B



55

Synthesizing examples of compound represented by Formula B are shown below.

## SYNTHESIZING EXAMPLE 4

## Synthesis of Compound 12B (m=0)

56

and 20 ml of water was further added and stirred for 30 minutes. Thereafter the liquid was subjected to filtration. The filtered precipitation was washed by about 40 ml of a mixture of methanol and water at a ratio of 1:1 and dried for one night at a temperature of from 50 to 60° C. Thus unpurified crystals were obtained.



Into a 100 ml four-mouth flask to which a nitrogen gas inlet pipe, a cooler, a thermometer and a stirrer were equipped, 1.96 g (0.075 moles) of potassium tert-butoxide 4 and 20 ml of tetrahydrofuran, hereinafter referred to as THF, were charged and stirred while introducing nitrogen gas.

A solution was prepared by dissolving 1.0 g (0.003 moles) of Compound 1 and 2.63 g (0.007 moles) of Compound 2 and 2.25 g (0.008 moles) of Compound 3 dissolved in 20 ml of THF. The solution was gradually dripped into the mixture of potassium tert-butoxide 4 and THF while the temperature was maintained at 45° C. After the finish of the dripping, reaction was carried out for 5 hours while maintaining a temperature of from 45 to 50° C.

To another 200 ml beaker, a stirrer was equipped and 20 ml of methanol was charged and stirred. The reaction liquid after the reaction for 5 hours was poured to the methanol,

50 The unpurified crystals were dissolved in 30 ml of toluene, and 3 g of Wakogel B-0, produced by Wako Pure Chemical Industries, Ltd., was added to the solution and stirred for 30 minutes and filtered. The Wakogel B-0 was washed by 30 ml of toluene. The filtrate and the washing toluene was concentrated and dried. The dried substance was dissolved by adding 10 ml of ethyl acetate. The solution was 55 dripped into 60 ml of methanol for purifying by re-precipitation. By filtering and drying, 3.20 g of a compound having the chemical structure 12B (m=0) was obtained.

As a result of analysis by high speed liquid chromatography and mass spectrography in the same manner as in 60 Synthesizing Example 1A, the above-obtained compound is a mixture of compounds having an n of from 0 to 5. The content ratio or area of high speed liquid chromatograph was n=0/1/2/3/4/5=24.3/44.4/21.5/7.2/2.3/0.3.

65 The determination condition of the high speed chromatography was carried out under the following conditions.

57

### SYNTHESIZING EXAMPLE 5

### Synthesis of Compound 11B (m=0)

58

washed by 30 ml of toluene. The filtrate and the washing toluene was concentrated and dried. The dried substance was dissolved by adding 10 ml of ethyl acetate. The solution was dripped into 60 ml of methanol for purifying by re-precipi-



Into a 100 ml four-mouth flask to which a nitrogen gas inlet pipe, a cooler, a thermometer and a stirrer were equipped, 1.96 g (0.075 moles) of potassium tert-butoxide 4 and 20 ml of tetrahydrofuran, hereinafter referred to as THF, were charged and stirred while introducing nitrogen gas.

A solution was prepared by dissolving 1.0 g (0.003 moles) of Compound 1 and 2.46 g (0.007 moles) of Compound 2 and 2.41 g (0.008 moles) of Compound 3 dissolved in 20 ml of THF. The solution was gradually dripped into the mixture of potassium tert-butoxide 4 and THF while the temperature was maintained at 45° C. After the finish of the dripping, reaction was carried out for 5 hours while maintaining a temperature of from 45° C. to 50° C.

To another 200 ml beaker, a stirrer was equipped and 20 ml of methanol was charged and stirred. The reaction liquid after the reaction for 5 hours was poured to the methanol, and 20 ml of water was further added and stirred for 30 minutes. Thereafter the liquid was subjected to filtration. The filtered precipitation was washed by about 40 ml of a mixture of methanol and water at a ratio of 1:1 and dried for one night at a temperature of from 50° C. to 60° C. Thus unpurified crystals were obtained.

The unpurified crystals were dissolved in 30 ml of toluene, and 3 g of Wakogel B-0, produced by Wako Pure Chemical Industries, Ltd., was added to the solution and stirred for 30 minutes and filtered. The Wakogel B-0 was

tation. By such filtering and drying, 3.35 g of a compound having the chemical structure of 11B ( $m=0$ ) was obtained.

As a result of analysis by high speed liquid chromatography and mass spectrography in the same manner as in Synthesizing Example 1A, the above-obtained compound is a mixture of compounds having an *n* of from 0 to 4. The content ratio or area of high speed liquid chromatograph was  $n=0/1/2/3/4=32.5/45.0/16.5/6.2/1.6$ .

The compounds represented by Formula C each have the following chemical structure.



In Formula C,  $\text{Ar}_1$  is a substituted or unsubstituted mono-valent aromatic group;  $\text{Ar}_6$  is a substituted or unsubstituted di-valent aromatic group, a di-valent heterocyclic group, or a group represented by Formula (8); and R is a substituted or unsubstituted alkyl group or a substituted or unsubstituted mono-valent aromatic group. Each of  $\text{Ar}_1$ ,  $\text{Ar}_6$  and R differs from each other.

**59**

In Formula (8),  $Z_3$  is an oxygen atom, a sulfur atom, a  $-\text{CH}=\text{CH}-$  group or a  $-\text{CH}_2-\text{CH}_2-$  group; and  $R_1$  and  $R_2$  are each a hydrogen atom or an alkyl group having from 1 to 4 carbon atoms.

In Formula C,  $\text{Ar}_1$  is a substituted or unsubstituted mono-valent aromatic group, and is preferably a substituted or unsubstituted phenyl group, a phenyl group substituted with an alkyl group having from 1 to 4 carbon atoms, or an alkoxy group.

**60**

The substituted of unsubstituted divalent aromatic group represented by  $\text{Ar}_6$  is preferably a phenylene group, a naphthylene group or a bi-phenylene group, and the substituent of them is preferably an alkyl group. As the di-<sup>5</sup>valent heterocyclic group represented by  $\text{Ar}_6$ , a di-<sup>2</sup>valent furan group or a di-<sup>2</sup>valent thiophene group are preferable.

Specific examples of the compound of Formula C

| Chemical structure<br>No. | $\text{Ar}_1$ | $\text{Ar}_6$ | $\text{R}$     |
|---------------------------|---------------|---------------|----------------|
| 1C                        |               |               |                |
| 2C                        |               |               |                |
| 3C                        |               |               |                |
| 4C                        |               |               | $\text{CH}_3-$ |
| 5C                        |               |               |                |
| 6C                        |               |               |                |
| 7C                        |               |               |                |
| 8C                        |               |               |                |
| 9C                        |               |               |                |

-continued

| Chemical structure No. | Ar <sub>1</sub> | Ar <sub>6</sub> | R |
|------------------------|-----------------|-----------------|---|
| 10C                    |                 |                 |   |
| 11C                    |                 |                 |   |
| 12C                    |                 |                 |   |
| 13C                    |                 |                 |   |
| 14C                    |                 |                 |   |
| 15C                    |                 |                 |   |
| 16C                    |                 |                 |   |
| 17C                    |                 |                 |   |
| 18C                    |                 |                 |   |
| 19C                    |                 |                 |   |

-continued

| Chemical structure No. | Ar <sub>1</sub> | Ar <sub>6</sub> | R                                                                                     |
|------------------------|-----------------|-----------------|---------------------------------------------------------------------------------------|
| 20C                    |                 |                 |                                                                                       |
| 21C                    |                 |                 |                                                                                       |
| 22C                    |                 |                 |                                                                                       |
| 23C                    |                 |                 |                                                                                       |
| 24C                    |                 |                 |                                                                                       |
| 25C                    |                 |                 |                                                                                       |
| 26C                    |                 |                 |                                                                                       |
| 27C                    |                 |                 |                                                                                       |
| 28C                    |                 |                 |                                                                                       |
| 29C                    |                 |                 |  |

-continued

| Chemical structure No. | Ar <sub>1</sub>                                                                     | Ar <sub>6</sub>                                                                     | R                                                                                     |
|------------------------|-------------------------------------------------------------------------------------|-------------------------------------------------------------------------------------|---------------------------------------------------------------------------------------|
| 30C                    |    |    |    |
| 31C                    |    |    |    |
| 32C                    |    |   |    |
| 33C                    |  |  | CH <sub>3</sub> —                                                                     |
| 34C                    |  |  |  |
| 35C                    |  |  |  |
| 36C                    |  |  |  |
| 37C                    |  |  |  |
| 38C                    |  |  |  |

-continued

| Chemical structure<br>No. | Ar <sub>1</sub> | Ar <sub>6</sub> | R |
|---------------------------|-----------------|-----------------|---|
| 39C                       |                 |                 |   |
| 40C                       |                 |                 |   |
| 41C                       |                 |                 |   |
| 42C                       |                 |                 |   |
| 43C                       |                 |                 |   |
| 44C                       |                 |                 |   |
| 45C                       |                 |                 |   |
| 46C                       |                 |                 |   |
| 47C                       |                 |                 |   |

-continued

| Chemical structure<br>No. | Ar <sub>1</sub> | Ar <sub>6</sub> | R                          |
|---------------------------|-----------------|-----------------|----------------------------|
| 48C                       |                 |                 |                            |
| 49C                       |                 |                 |                            |
| 50C                       |                 |                 |                            |
| 51C                       |                 |                 |                            |
| 52C                       |                 |                 |                            |
| 53C                       |                 |                 |                            |
| 54C                       |                 |                 |                            |
| 55C                       |                 |                 |                            |
| 56C                       |                 |                 | $(\text{CH}_3)_3\text{C}-$ |

71

The synthesizing example of compounds represented by Formula C is described below.

## SYNTHESIZING EXAMPLE 6

## Synthesize of Compound 17C

Into a 100 ml four-mouth flask to which a nitrogen gas inlet pipe, a cooler, a thermometer and a stirrer were equipped, 4.08 g (0.04 moles) of 2,4-dimethylaniline, 4.08 g (0.02 moles) of iodobenzene, 9.9 g (0.03 moles) of diiodobenzene, 1.27 g (0.02 moles) of powdered copper and 11.04 g (0.08 moles) of potassium carbonate were charged and reacted over 30 hours at 190° C. while introducing nitrogen gas.

The reaction liquid was cooled to 60° C. and 200 ml of THF was added to the liquid, and the mixture was filtered. The filtrate was concentrated and dissolved in 100 ml of toluene and 10 g of Wakogel B-0 (Wako Pure Chemical Industries, Ltd.) was added, and stirred for 30 minutes and filtered. Filtered Wakogel was washed by 30 ml of toluene. The filtrate and the washing liquid were concentrated and dried. The dried substance was dissolved in 20 ml of THF and the solution was dripped into 120 ml of methanol for purifying by re-precipitation. The precipitate was filtered and dried, thus 5.15 g of Compound 17C was obtained.

According to the results of the analysis by high speed liquid chromatography and mass spectrography, the above-obtained compound has a composition of  $n=0/1/2/3/4/5/6/7=2.7/9.0/24.3/34.2/20.1/7.8/1.7/0.2$ . The weight average molecular weight (in terms of polystyrene) Mw of the compound measured via gel permeation chromatography (GPC) was 910.

## Synthesizing Example 7

## Synthesis of Compound 48C

Charged into a 100 ml four-mouth flask equipped with a nitrogen gas inlet pipe, a cooler, a thermometer and a stirrer, were 6.05 g (0.05 moles) of 2,4-dimethylaniline, 5.60 g (0.02 moles) of iodobiphenyl, 13.11 g (0.04 moles) of bis(4-bromophenyl) ether, 1.59 g (0.025 moles) of copper powder and 13.8 g (0.1 moles) of potassium carbonate were charged and reacted for 30 hours at 190° C. while introducing nitrogen gas.

The reacting liquid was cooled to 60° C. and 200 ml of THF was added to the liquid and the mixture was filtered. The filtrate was concentrated and dissolved by 100 ml of toluene and 10 g of Wakogel B-0 (Wako Pure Chemical Industries, Ltd.) was added, and stirred for 30 minutes and filtered. Filtered Wakogel was washed with 30 ml of toluene. The filtrate and the washing liquid were concentrated and dried. The dried substance was dissolved by adding 20 ml of THF, and the solution was dripped into 120 ml of methanol for purifying by re-precipitation. The precipitate was filtered and dried, whereby 10.56 g of Compound 48C was obtained.

Based on the results of analysis via high speed liquid chromatography and mass spectrography, the above-obtained compound has a composition of  $n=0/1/2/3/4/5/6/7/8=0.9/3.4/12.0/22.8/31.3/19.9/6.9/2.5/0.3$ . The weight average molecular weight in terms of polystyrene Mw of the compound measured by gel permeation chromatography (GPC) was 1684.

The charge transfer material according to the invention contains the mixture of compounds represented by Formula (1) in which n has a range of distribution and (Rp+Rs) is not

72

more than 99% when Rp represents the ratio of a component having the maximum content in the mixture and Rs represents the ratio of a component having the content next to the maximum content. The value of (Rp+Rs) is preferably from 30% to 99%, and more preferably from 45% to 90%. When (Rp+Rs) is less than 30%, the distribution of n becomes too broad and the molecular weight tends to be larger so that solubility and compatibility of the solvent or the binder resin tend to be degraded. When (Rp+Rs) is more than 99%, in the 10 case of the ratio of the low molecular component is lowered, the solubility and the compatibility with the solvent or the binder resin tend to be degraded also.

The value of n is from 0 to 10, but a composition having an n of 11 or more may be viable. It is acceptable that the 15 component of maximum content in the mixture and that of content next to the maximum content are within the range of from 0 to 10 and (Rp+Rs) is not more than 99%.

The average molecular weight of the mixture of compounds is preferably from 650 to 2,500, and more preferably from 800 to 2,300. The average molecular weight is represented by the weight average molecular weight in terms of polystyrene. When the average molecular weight exceeds 2,500, solubility in the solvent and compatibility with the binder resin of the charge transfer layer are degraded. As a 20 result of that, the dispersibility of the charge transfer material is lowered and electrophotographic properties of the photoreceptor such as the sensitivity and the charge uniformity are considerably degraded. When the average molecular weight is less than 650, properties of the layer such as the glass transition point Tg is degraded, and the black spotting and the recurring image defects tend to be observed.

The layer structure of the electrophotographic photoreceptor, particularly the organic photoreceptor, containing the mixture of compounds according to the invention is 30 described below.

The organic photoreceptor to be used in the invention is 35 described below.

## Electroconductive Substrate

Both a sheet-shaped substrate and a cylindrical substrate may be used as the electroconductive substrate of the photoreceptor. The cylindrical electroconductive substrate is 40 preferred for actuating a compact image forming apparatus.

The cylindrical electroconductive substrate is a cylinder-shaped substrate capable of endlessly forming an image, and such the substrate preferably has a linearity of not more than 45 0.1 mm and a fluctuation of not more than 0.1 mm.

A metal drum made from a metal such as aluminum and 50 nickel, a plastic drum on which a conductive substance such as aluminum, tin oxide and indium oxide is evaporated and a paper or plastic drum on which a electroconductive material is coated, may be used as the electroconductive drum. The electroconductive substrate having a specific conductivity of not less than  $10^3$   $\Omega\text{cm}$  is preferred.

An electroconductive substrate on which an anodized and 55 sealed layer is provided may also be used. The anodizing treatment is usually performed in an acidic bath such as chromic acid, sulfuric acid, oxalic acid, phosphoric acid, boric acid and sulfamic acid, and the treatment by the sulfuric acid bath is preferable. In the case of the anodizing in the sulfuric acid bath, a sulfuric acid concentration of from 100 to 200 g/L, an aluminum ion concentration of from 1 to 10 g/L, a bath temperature of about 20° C. and an applying voltage of about 20 V are preferred. The average thickness of the anodized layer is usually not more than 20  $\mu\text{m}$ , and preferably not more than 10  $\mu\text{m}$ .

## Interlayer

An interlayer (including a subbing layer) may be provided between the substrate and the photosensitive layer to improve the adhesiveness between the electroconductive substrate and the photosensitive layer and to prevent the injection of charge from the substrate. As the interlayer material, polyamide resin, vinyl chloride resin, vinyl acetate and copolymer containing at least two of the repeating unit of the above-mentioned resin are usable. Among the resins, polyamide resin is preferred since the residual charge accompanying repeated use of the photoreceptor can be reduced by the use of polyamide resin. The thickness of the interlayer using such the resin is preferably from 0.01 to 0.5  $\mu\text{m}$ .

An interlayer made from a hardenable metal resin is also preferred, and is commonly prepared by a thermally hardening of an organic metal compound such as a silane coupling agent and a titanium coupling agent. The thickness of the interlayer of hardenable metal resin is preferably from 0.1 to 2  $\mu\text{m}$ .

An interlayer composed of a binder resin in which an organic particle is also preferably usable. The average diameter of the inorganic particles is preferably from 0.01 to 1  $\mu\text{m}$ . An interlayer composed of a binder resin in which surface treated N-type semi-conductive fine particle is dispersed is particularly preferred. For example, an interlayer composed of polyamide resin and titanium oxide treated with silica-alumina compound and a silane having an average diameter of from 0.01 to 1  $\mu\text{m}$  dispersed in the polyamide resin is particularly preferred. The thickness of such an interlayer is preferably from 1 to 20  $\mu\text{m}$ .

The N-type semi-conductive fine particle is a fine particle in which an electron functions as the electroconductive carrier. The particle contained in the insulation resin effectively blocks holes injected from the substrate and does not block electrons from the photosensitive layer.

A method to confirming the N-type semi-conductive particle is described below.

An interlayer of 5  $\mu\text{m}$  was prepared on an electroconductive substrate using a dispersion prepared by dispersing particles in a binder resin at a ratio of 50% by weight. The interlayer is negatively charged and the photo-decay of the charge measured. Alternatively, the interlayer is positively charged and the photo-decay of the charge can be measured.

When the photo-decay of the negative charge is greater than that of the positive charge, the particle is an N-type semi-conductive particle.

Examples of the particles include titanium oxide  $\text{TiO}_2$ , zinc oxide  $\text{ZnO}$  and tin oxide  $\text{SnO}_2$ . Preferably used in the invention is titanium oxide.

The average diameter of minute N-type semi-conductive particles is preferably from 10 nm to 500 nm, more preferably from 10 nm to 200 nm, and further preferably from 15 nm to 200 nm, in the number average diameter of the primary particles.

By the use of the fine particle having such the average diameter, high density and uniform dispersion of the particles in the interlayer can be attained to give sufficient charge stability and the black spotting preventing function to the interlayer.

In the case of titanium oxide, for example, the number average of the diameter of the primary particles of the N-type semi-conductive fine particle is determined as the number average of the Fere diameter obtained by image analysis of image of randomly selected 100 primary particles employing a transmission electron microscope at a magnification of 10,000.

The N-type semi-conductive fine particles possess various shapes such as branch-like, needle-like and grain-like. For example, the crystal type of titanium oxide includes anatase type, rutile type and amorphous type. Any type may be used and two or more crystal types may be used in combination. Of them, the rutile type is most preferable.

It is preferable that the N-type semi-conductive fine particle is used after a hydrophobilizing surface treatment. In one of the hydrophobilizing surface treatment, plural surface treatments are performed, and the last treatment is carried out using a reactive organic silicon compound. It is preferred that, at least one of the plural treatments is performed by at least one of alumina, silica and zirconia and the last treatment is carried out by the reactive organic silicon compound.

The alumina, silica and the zirconia treatments are each a treatment to precipitate alumina, silica and zirconia onto the surface of the N-type semi-conductive fine particle, respectively. The alumina, silica and zirconia precipitated onto the fine particles each contains hydrated compound of alumina, silica and zirconia, respectively. The surface treatment via the reactive organic silicon compound is performed by using a treatment solution containing a reactive organic silicon compound.

The surface of N-type semi-conductive fine particle such as the titanium oxide particle is uniformly covered by at least two repeated surface treatments. The surface of the treated N-type semi-conductive fine particle shows high dispersibility in the interlayer, and results in a good photoreceptor without occurrence of image defects such as the black spotting can be obtained.

The photoreceptor may be a single layer photoreceptor in which a layer having both functions of charge generation and charge transfer is provided on an interlayer. However, it is preferable that the function of the photosensitive layer is separated into a charge generation layer CGL and a charge transfer layer CTL. By such a separation, the increase of the residual potential accompanying repeated use can be controlled to low levels and other electrophotographic properties can also be easily controlled depending on the purpose. In a photoreceptor to be negatively charged, it is preferred that the CGL is provided on the interlayer and the CTL is provided on the CGL. In a photoreceptor to be positively charged, the CTL is provided on the interlayer and the CGL is provided on the CTL. In the invention, the negatively charged photoreceptor having a function separated structure is most preferable.

The layer arrangement of the function separated type negatively charged photoreceptor is described below.

## CGL

CGL contains a charge generation material, CGM. A binder resin and another additive may be incorporated based on the desired function.

Examples of the CGM include a phthalocyanine dye, an azo dye, a perylene dye and an azurenium dye. Of these a CGM having a crystal structure capable of assuming a stable aggregated structure among plural molecules thereof is most effective to inhibit an increase of residual potential accompanying repeated use. Specifically, CGM of a phthalocyanine dye and perylene dye each having a specific crystal structure are exemplified. For example, CGM of tianylphthalocyanine having a maximum peak of Bragg angle 20 of diffraction of Cu-K $\alpha$  X-ray at 27.2°, and benzimidazoleperylene having a maximum peak of the 20 angle at 12.4° show almost no degradation accompanying repeated use and make the residual potential to small.

A resin can be used as the dispersing medium of the CGL or the CTL. Examples of preferable resins include a formal resin, a butyral resin, a silicone resin, a silicone-modified butyral resin and a phenoxy resin. By the use of such the resins, the increase of residual potential accompanying repeated use can be most inhibited. The ratio of the charge generation material to the binder resin is preferably from 20 to 600 parts by weight per 100 parts by weight of the binder resin. The thickness of the charge generation layer is preferably from 0.01 to 2  $\mu\text{m}$ .

## CTL

CTL contains the charge transfer material CTM and a binder resin for dispersing the CTM and for forming layer. An additive such as an antioxidant may be contained according to necessity.

As the CTM, a mixture of two or more kinds of compounds each represented by Formula (1) may be used, each of which has the average molecular weight of not more than 2,500, and different from each other in the  $n$  value of Formula (1). In addition, for example, a triphenylamine derivative, a hydrazone compound, a styryl compound, a benzidine compound and a butadiene compound may be

used together. The charge transfer material is usually dissolved in a suitable resin for forming the layer.

Examples of resin to be used for CTL include a polystyrene resin, an acryl resin, a methacryl resin, a vinyl chloride resin, a vinyl acetate resin, a polyvinyl butyral resin, an epoxy resin, a polyurethane resin, a phenol resin, a polyester resin, an alkyd resin, a polycarbonate resin, a silicone resin, a melamine resin and a copolymer containing two or more repeating units of the above-listed resins. Other than the forgoing insulation resin, an organic semi-conductive material such as poly-N-vinylcarbazole is also usable.

Of these, polycarbonate resin is most preferable as the binder from the viewpoint of the dispersibility of the CTM and electrophotographic properties. The ratio of the charge transfer material to the binder is preferably from 10 to 200 parts by weight per 100 parts by weight of the binder resin.

It is preferable that the CTL contains an antioxidant. The antioxidant prevents or inhibits the action caused by lighting, heating or discharging to an auto-oxidizable substance being at interior or surface of the photoreceptor. Typical examples of the antioxidant are as follows.



-continued

1-9

1-10



2-1



2-2



2-3



2-4

2-5



2-6



-continued



The charge transfer layer may be constituted by two or more layers. In such case, the surface charge transfer layer satisfies the requirements of the invention. The thickness of the charge transfer layer is preferably from 10 to 40  $\mu\text{m}$ .

Examples of the solvent or the dispersing medium for forming the photosensitive layer, interlayer and surface layer include n-butylamine, diethylamine, ethylenediamine, iso-propanolamine, triethanolamine, triethylenediamine, N,N-dimethylformamide, acetone, methyl ethyl ketone, methyl isopropyl ketone, cyclohexanone, benzene, toluene, xylene, chloroform, dichloromethane, 1,2-dichloroethane, 1,2 dichloropropane, 1,1,2-trichloroethane, 1,1,1-trichloroethane, trichloroethylene, tetrachloroethane, tetrahydrofuran, dioxolane, dioxane, methanol, ethanol, butanol, isopropanol, ethyl acetate, butyl acetate, dimethylsulfoxide and methyl cellosolve. Dichloromethane, 1,2-dichloroethane and methyl ethyl ketone are preferably used even though the invention is not limited to the above-mentioned. These solvent may be used solely or as a mixture of two or more kinds thereof.

The coating liquids for the layers are preferably filtered with such as a metal filter or a membrane filter before the coating thereof to remove foreign matters or an aggregate. It is preferable that the filter is selected from filters such as a pleated type filter (HDC), a depth type filter (Profile), each manufactured by Nihon Paul Co., Ltd. and a semi-depth type filter (Profilestar) based on the properties of the coating liquid.

A coating method such as an immersion coating method, a spray coating method or a circular coating amount controlling type coating method is usable for producing the organic electrophotographic photoreceptor. The spray coating method or the coating method using a circular coating amount controlling coating type coater, being typically a circular slide hopper coater, is preferably applied for coating the upper layer of the photosensitive layer since dissolving of the lower layer can be inhibited to remain as small as possible and a uniform coated layer can be formed by such a coating method. The circular coating amount controlling type coater is preferably applied for the coating of the protective layer. The circular coating amount controlling coater is described in, for example, JP O.P.I. Publication No. 58-189061.

The image forming method and the image forming apparatus using the photoreceptor according to the invention are described below.

FIG. 1 shows a cross section of the structure of an image forming apparatus as an example of the image forming method according to the invention.

In FIG. 1, numeral 50 is a photoreceptor drum as an image carrier which is a photoreceptor comprising a drum and an organic photosensitive layer coated on the drum; the drum is grounded and driven to be clockwise rotated. 52 is a

15 scorotron charging device as a charging unit which provides uniform charge onto the circumferential surface of the photoreceptor drum 50 by corona discharge. The residual charge on the drum surface may be removed before charging by charging device 52 by using pre-exposing device 51 20 having a light emission diode for erasing the charge history.

After uniformly charging the photoreceptor, image exposure based on the image information is provided by image exposure device 53 as an image exposing means. The light source of the exposing device 53 is a laser diode which is not shown in the drawing. A latent static image is formed by scanning via light beam along the optical path introduced by reflection mirror 532 through rotating polygon mirror 531 and an f0 lens.

30 The reversal developing process is a developing process in which the photoreceptor surface is uniformly charged by charging device 52 and the potential of the image exposed area or the exposed area potential is visualized by a developing unit. Alternatively, the unexposed area is not visualized by the bias potential applied to developing sleeve 541.

35 Then the latent static image is developed by a developing device 54 as a developing unit. Developing device 54 including a developer comprising a toner and a carrier is arranged around photoreceptor drum 54, and the development is performed by developing sleeve 541 incorporating a magnet and rotated while holding the developer. The interior of the developing device 54 is constituted by a developer stirring and conveying member 544 and 543 and a conveying developer amount regulation member 542, whereby the developer is stirred, conveyed and supplied to the developing sleeve. The supplied amount of the developer is regulated by conveying amount regulating member 542. The conveyed amount of the developer is usually from 20 to 200 mg/cm<sup>2</sup> even though the amount may vary depending on the line speed of the electrophotographic photoreceptor and the specific gravity of the developer.

40 The developer is composed of the carrier, the toner and the external additive. The carrier is composed of a ferrite core coated with an insulation resin, and the toner is composed of a colored particle comprising the styrene-acryl resin as the principal component, the charge controlling agent and low molecular weight polyolefin. Examples of the 45 external additive include silica and titanium oxide. The developer is conveyed into the developing zone while the layer thickness thereof is regulated by the conveying toner amount regulating member, and the development is performed. At this time, the development is usually performed while applying direct current bias, and alternative current bias based on necessity, between the photoreceptor drum and developing sleeve 541. Development is performed in the 50 status in which the developer is contact or not in contact with the photoreceptor. The electrical potential of the photore-

ceptor is measured by a potential sensor installed at the upper portion of the developing zone.

Recording paper P is synchronously supplied into the transfer zone by the rotation of a paper supplying roller 57 in timing of transfer after the image formation.

In the transfer zone, transfer electrode 58 synchronously acts on the circumference of the photoreceptor drum in time with the transfer to apply charge having the reversed polarity of the toner to recording paper P to which the toner transfers.

The charge of recording paper P is neutralized by a separation electrode or separating device 59, and the recording paper P is separated from the circumference of the photoreceptor drum 59 after which it is conveyed into fixing device 60. In the fixing device the toner is fused and fixed onto the paper by heating and pressing by a heating roller 601 and a pressing roller 602 and ejected out from the apparatus through ejecting roller 61. Transfer electrode 58 and separation electrode 59 are temporarily stopped after passing of recording paper P for preparing to the subsequent image formation. In FIG. 1, a scorotron transfer electrode is used. Conditions of the transfer electrode are set at, for example, a transfer current of from +100 to +400  $\mu$ A and a transfer voltage of from +500 to +2,000 V even though the conditions cannot be simply limited since the conditions vary depending on the processing speed or circumferential rate of the photoreceptor.

Toner remaining on photoreceptor drum 50 after the separation of recording paper P is removed, and the drum surface is cleaned by cleaning blade 621 of a cleaning device or cleaning unit 62 pressed onto the drum, which is then subjected to exposure before charging by pre-exposing device 51 and to charging by charging device 52. Thus photoreceptor drum 50 enters the next image forming cycle.

Numerical 70 is a processing cartridge capable of being freely installed in and released from the apparatus, in which the photoreceptor, the charging device, the transferring device, the separation device and the cleaning device are integrated.

The electrophotographic photoreceptor according to the invention is suitable for an electrophotographic photoreceptor, a laser printer, an LED printer and a liquid crystal shutter type printer. Further, the photoreceptor can be widely applied to an apparatus utilizing electrophotographic technology for display, recording, light printing, plate making and facsimile.

## EXAMPLES

The present invention is described in detail referring to the examples below. In the following, "part" means "parts by weight".

### Example 1

Photoreceptors containing a mixture of compounds represented by Formula A were prepared as follows.

#### Preparation of Photoreceptor 1A

##### <Interlayer>

|                                                                                                                                              |           |
|----------------------------------------------------------------------------------------------------------------------------------------------|-----------|
| Polyamide resin, Amilan CM-8000 (Toray Co., Ltd.)                                                                                            | 60 parts  |
| Inorganic fine particles, titanium oxide SMT500SAS (Tayca Corporation, surface treated by silica, alumina, and methyl hydrogen polysiloxane) | 180 parts |

-continued

|           |            |
|-----------|------------|
| Methanol  | 1600 parts |
| 1-butanol | 400 parts  |

The above components were mixed and dissolved to prepare an interlayer coating liquid. The coating liquid was coated by an immersion method on the cylindrical aluminum substrate and dried. Thus a 1.0  $\mu$ m interlayer was prepared.

##### <Charge Generation Layer>

|                                                                                                                           |           |
|---------------------------------------------------------------------------------------------------------------------------|-----------|
| 15 Titanylphthalocyanine (The highest peak of Bragg angle 20 of 27.3° for Cu-K $\alpha$ characteristic X-ray diffraction) | 60 parts  |
| Silicone resin solution, 15% xyrene/butanol solution of KRS240 (Shin'etsu Kagaku Co., Ltd.)                               | 700 parts |

The above components were mixed and dispersed for 10 hours using a sand mill to prepare a charge generation layer coating liquid. The coating liquid was coated onto the interlayer by the immersion method and dried. Thus a 0.3  $\mu$ m charge generation layer was formed.

##### <Charge transfer layer>

|                                                                                                   |            |
|---------------------------------------------------------------------------------------------------|------------|
| 30 Charge transfer material (Compound of Synthesizing Example 1)                                  | 150 parts  |
| Binder resin, bis-phenol Z type polycarbonate Eupiron Z300 (Mitsubishi Gas Chemical Company Inc.) | 300 parts  |
| Antioxidant, Sanol LS2626 (Sankyo Co., Ltd.)                                                      | 1.7 parts  |
| Tetrahydrofuran                                                                                   | 2000 parts |

The above components were mixed and dissolved to prepare a charge transfer layer coating liquid. The coating liquid was applied onto the charge generation layer by the immersion method and dried for 40 minutes at 100°C. to form a 22  $\mu$ m charge transfer layer, whereby Photoreceptor 1A was prepared.

##### Preparation of Photoreceptors of 2A through 14A

Photoreceptors 2 through 14A were prepared in the same manner as Photoreceptor 1A except that the charge generation compound, the charge transfer compound, the amounts of the compounds, and the thickness of the charge transfer layer were altered as shown in Table 1.

##### Preparation of Photoreceptor 15A

Photoreceptor 15A was prepared in the same manner as Photoreceptor 1A except that the charge transfer material or the compound of Synthesizing Example 1 was replaced by the component n=0 of Compound 21A (p=0, q=0) synthesized by a commonly known method. The purity of the component was greater than 99%.

##### Preparation of Photoreceptor 16A

Photoreceptor 16A was prepared in the same manner as Photoreceptor 1A except that the charge transfer material or the compound of Synthesizing Example 1 was replaced by the n=3 component of Compound 21A (p=0, q=0) separated by liquid chromatography from the compound of Synthesizing Example 1. The purity of the component was larger than 99%. However, any photoreceptor capable of being evaluated cannot be obtained since the compound was not permissible with the binder resin and precipitated.

## Preparation of Photoreceptor 17A

The compound of Synthesizing Example 1 was separated by liquid chromatography into each component and a mixture of 50% of the n=1 component and 50% of n=2 of Compound 21A (p=0, q=0) was prepared. Then Photoreceptor 17A was prepared in the same manner as Photoreceptor 1A except that the charge transfer material was replaced by the above mixture.

evaluation was basically performed on 10,000 copied sheets by an intermittent mode. Used an original image for the copying test was a A4 size image including a texture image at a pixel ratio of 7%, a halftone image, a solid white image and a solid black image each occupying one fourth of the original image area. Results of the evaluation are shown in Table 4.

TABLE 1

| Photoreceptor No. | Charge material | layer generation | Charge transfer layer                                      |                    |      |      |       |       |       |       |       |       |       |       | Average molecular weight (Mw) | Amount (parts) | Layer thickness Re- (μm) | Remarks |  |  |  |
|-------------------|-----------------|------------------|------------------------------------------------------------|--------------------|------|------|-------|-------|-------|-------|-------|-------|-------|-------|-------------------------------|----------------|--------------------------|---------|--|--|--|
|                   |                 |                  | Charge transfer material (Compound and constitution ratio) |                    |      |      |       |       |       |       |       |       |       |       |                               |                |                          |         |  |  |  |
|                   |                 |                  | Charge generation No.                                      | Chemical structure | p    | q    | n = 0 | n = 1 | n = 2 | n = 3 | n = 4 | n = 5 | n = 6 | n = 7 | n = 8                         |                |                          |         |  |  |  |
| 1A                | Y               | 21A              | 0                                                          | 0                  | 27.4 | 44.8 | 20.1  | 6.3   | 1.4   | 0.0   | 0.0   | 0.0   | 0.0   | 72.2  | 1475                          | 150            | 22                       | Inv.    |  |  |  |
| 2A                | Y               | 21A              | 1                                                          | 0                  | 33.4 | 46.8 | 15.0  | 4.0   | 0.8   | 0.0   | 0.0   | 0.0   | 0.0   | 80.2  | 1314                          | 150            | 22                       | Inv.    |  |  |  |
| 3A                | Y               | 14A              | 1                                                          | 0                  | 30.1 | 45.4 | 16.7  | 6.0   | 1.8   | 0.0   | 0.0   | 0.0   | 0.0   | 75.5  | 1194                          | 150            | 22                       | Inv.    |  |  |  |
| 4A                | Y               | 21A              | 0                                                          | 0                  | 27.4 | 44.8 | 20.1  | 6.3   | 1.4   | 0.0   | 0.0   | 0.0   | 0.0   | 72.2  | 1475                          | 225            | 27                       | Inv.    |  |  |  |
| 5A                | Y               | 21A              | 0                                                          | 0                  | 27.4 | 44.8 | 20.1  | 6.3   | 1.4   | 0.0   | 0.0   | 0.0   | 0.0   | 72.2  | 1475                          | 100            | 16                       | Inv.    |  |  |  |
| 6A                | Y               | 12A              | 0                                                          | 0                  | 54.0 | 31.3 | 10.3  | 3.5   | 0.9   | 0.0   | 0.0   | 0.0   | 0.0   | 85.3  | 991                           | 150            | 22                       | Inv.    |  |  |  |
| 7A                | Y               | 16A              | 0                                                          | 0                  | 31.5 | 46.0 | 16.0  | 5.3   | 1.2   | 0.0   | 0.0   | 0.0   | 0.0   | 77.5  | 1426                          | 150            | 22                       | Inv.    |  |  |  |
| 8A                | Z               | 22A              | 0                                                          | 0                  | 21.1 | 43.8 | 22.0  | 9.8   | 3.0   | 0.0   | 0.0   | 0.0   | 0.0   | 65.8  | 1663                          | 150            | 22                       | Inv.    |  |  |  |
| 9A                | Z               | 36A              | 0                                                          | 0                  | 33.7 | 34.0 | 19.8  | 9.6   | 2.7   | 0.2   | 0.0   | 0.0   | 0.0   | 67.7  | 1739                          | 150            | 22                       | Inv.    |  |  |  |
| 10A               | Y               | 15A              | 0                                                          | 1                  | 29.6 | 41.1 | 20.5  | 7.6   | 1.2   | 0.0   | 0.0   | 0.0   | 0.0   | 70.7  | 1520                          | 150            | 22                       | Inv.    |  |  |  |
| 11A               | Y               | 12A              | 1                                                          | 1                  | 19.8 | 36.1 | 28.6  | 10.4  | 4.1   | 1.0   | 0.0   | 0.0   | 0.0   | 64.7  | 1892                          | 150            | 22                       | Inv.    |  |  |  |
| 12A               | Y               | 21A              | 0                                                          | 0                  | 5.8  | 13.0 | 21.0  | 22.2  | 17.5  | 11.1  | 6.1   | 3.0   | 0.3   | 43.2  | 2282                          | 150            | 22                       | Inv.    |  |  |  |
| 13A               | Y               | 21A              | 0                                                          | 0                  | 12.7 | 25.9 | 30.3  | 18.1  | 9.2   | 2.9   | 0.9   | 0.0   | 0.0   | 56.2  | 1869                          | 150            | 22                       | Inv.    |  |  |  |
| 14A               | Y               | 21A              | 0                                                          | 0                  | 65.4 | 28.9 | 5.2   | 0.5   | 0.0   | 0.0   | 0.0   | 0.0   | 0.0   | 94.3  | 908                           | 150            | 22                       | Inv.    |  |  |  |
| 15A               | Y               | 21A              | 0                                                          | 0                  | 100  | 0.0  | 0.0   | 0.0   | 0.0   | 0.0   | 0.0   | 0.0   | 0.0   | 100   | 643                           | 150            | 22                       | Comp.   |  |  |  |
| 16A               | Y               | 21A              | 0                                                          | 0                  | 0.0  | 0.0  | 0.0   | 100   | 0.0   | 0.0   | 0.0   | 0.0   | 0.0   | 100   | 1882                          | 150            | 22                       | Comp.   |  |  |  |
| 17A               | Y               | 21A              | 0                                                          | 0                  | 0.0  | 50   | 50    | 0.0   | 0.0   | 0.0   | 0.0   | 0.0   | 0.0   | 100   | 1263                          | 150            | 22                       | Comp.   |  |  |  |

Inv.; Inventive

Comp.; Comparative

In the above table, Y is titanylphthalocyanine pigment (in which the highest peak of a Bragg angle  $2\theta$  is  $27.3^\circ$  of a Cu-K $\alpha$  characteristic X-ray diffraction spectrogram).

Z is bemzimidazoleperylene pigment (the highest peak of a Bragg angle  $2\theta$  is  $12.4^\circ$  of a Cu-K $\alpha$  characteristic X-ray diffraction spectrogram).

(Rp+Rs) is the sum of the content in percent of the compound having the maximum content in the mixture and the content in percent of the compound having the content next to the maximum content.

The distribution or content ratio of n of the chain structure of the charge transfer material is determined based on the ratio of the area of high speed liquid chromatograph GPC. The average molecular weight, Mw, is the weight average molecular weight in terms of polystyrene determined via gel permeation chromatography.

## Evaluation

The above-obtained Photoreceptors 1A through 17A were each installed into a digital copying machine utilizing reversal development system Konica 7085, manufactured by Konica Corp., and subjected to the following evaluation. The copying machine had a scorotron charging device, a semi-conductor laser exposing device emitting 680 nm light, a reversal developing unit and a printing rate of 85 sheets of A4 size paper per minute. Evaluation was carried out under an environmental conditions, or temperature and moisture conditions based on each of the evaluation items. The

## Evaluation Condition

Line speed: 420 mm/second

Duration between the imagewise exposure and the developing position: 0.108 second

## Charging Condition

Charging device: Scorotron charging device for negative charging

Charging potential: -700 V to -750 V

## Exposure Condition

Exposure amount was set so that the potential of the solid black image portion was -100 V.

A developer composed of a ferrite carrier coated with an insulation resin and a toner composed of a colored particles and silica and titanium oxide added as the external additive was used. The colored particle had a volume average diameter of  $5.3 \mu\text{m}$  and contained a styrene-acryl resin as the principal component, carbon black as the colorant, a charge controlling agent and a low molecular weight polyolefin. The colored particles were prepared via a polymerization method.

## Transferring Condition

Transferring electrode: Corona charging electrode for positive charging

## Separation Condition

A separating unit of a separation claw unit was used.

## Cleaning Condition

A cleaning blade having a hardness of  $70^\circ$ , a repulsive elasticity of 65%, a thickness of 2 mm and a free length of 9 mm was placed onto the photoreceptor in the counter

85

clockwise direction and a line pressure of 18 g/cm was applied by a weight loading system.

#### Evaluation Items and Methods

Evaluation was carried out at high speed response or electrical potential variation of the solid black image area under a low temperature and low humidity condition of 10° C. and 20% RH.

Copying of 10,000 sheets by an intermittent mode was performed under the above low temperature-humidity condition. Used as the original image for the copying test was a A4 size image including text at a pixel ratio of 7%, a halftone image, a solid white image and a solid black image each occupying one fourth of the original image area. The difference of the electrical potential at initiation of printing and that after 10,000 sheets of copying of the solid black image area  $|\Delta V|$  was measured. A smaller value of  $|\Delta V|$  corresponds to a higher high-speed response under the low temperature and low moisture condition of 10° C. and 20% RH, respectively.

A: The electrical potential variation of the solid black image area  $|\Delta V|$  was less than 50V; rated as good.

B: The potential variation at the solid black image area  $|\Delta V|$  is from 50 V to 150 V; rated as no problem for practical use.

C: The potential variation at the solid black image area  $|\Delta V|$  was more than 150V; rated as potential problems in the practical use.

Thinning of texture image under low temperature and low humidity condition of 10° C. and 20% RH.

An original image on which line at a width of 0.1 mm and 0.2 mm was copied for evaluation.

A: In the copied image, the width of reproduced line was not less than 75% of the original image; rated as good.

B: In the copy image, the width of reproduced line was from 40% to 74% of the original image; rated as no problem for the practical use.

C: In the copy image, the width of reproduced line was not more than 39% of that of the original image or the line image was broken; rated as a potential problem in practical use.

Black Spotting under a High Temperature and High Humidity Condition of 30° C. and 80% RH

The occurrence of the black spotting (strawberry seed like shaped spotted image) on the halftone image was evaluated according to the following norms.

A: No black spotting forming nucleus was observed on the photoreceptor and no black spotting observed on the halftone image; rated as good.

B: No black spotting occurred on the halftone image even though black spotting forming nuclei observed on the photoreceptor; rated as no problem for practical use.

C: Black spotting forming nuclei were observed on the photoreceptor and black spotting occurred on the halftone image; rated as a potential problem in practical use.

Occurrence of recurring image defects under a high temperature and high humidity condition of 30° C. and 80% RH

Evaluated was number of visible recurring defect such as a white image lacking, black spotting and line-shaped defects wherein synchronous with the period of rotation of the photoreceptor.

86

A: Frequency of image defects of not less than 0.4 mm was not more than 5 per A4 size image in the entire copies; rated as good.

B: Frequency of the image defect of not less than 0.4 mm was that at least one sheet having 6 to 10 defects per A4 size image was found; rated as no problem for practical use.

C: Frequency of the image defect of not less than 0.4 mm was that at least one sheet having not less than 11 defects per A4 size image was found; rated as a potential problem in practical use.

#### Cracking

The power source was turned to the digital copying machine Konica 7085 in which the photoreceptors to be evaluated were installed, and stood idle for 2 days under a condition of 30° C. and 80% RH. During the idling for 2 days, the devices around the photoreceptor were stayed at the condition when the action was stopped, namely the cleaning blade and the developer conveying member remained in the contacted state to the photoreceptor. Thereafter, the occurrence of the cracking on the surface of the photoreceptor was observed, in addition, the occurrence of linear image defects accompanying the occurrence of cracking was also evaluated.

A: One hundred photoreceptors were evaluated but no cracking nor image defect were found; rated as good.

B: One hundred photoreceptors were evaluated and slight cracking was found but no image defect was observed; rated as no problem for practical use.

C: One hundred photoreceptors were evaluated and cracking and the line-shaped image defects were observed; rated as potential a problem in practical use.

Image Density under the Low Temperature and Low Humidity Condition of 10° C. and 20% RH

The reflective density of a solid black image was measured via RD-918, manufactured by Macbeth Co., Ltd. The evaluation was performed according to the relative density when the density of an A4 size paper sheet before copying was set at 0.00.

A: Not less than 1.2; rated as good.

B: Not less than 1.2 to 0.8; rated as no problem for practical use.

C: Less than 0.8; rated as a potential problem in practical use.

#### Sharpness

Images of 3 and 5 point characters formed under low temperature and humidity condition of 10° C. and 20% RH respectively and that formed under a high temperature and humidity condition of 30° C. and 80% RH were evaluated for spreading of the text images according to the following norms.

A: Both of the images of the 3 and 5 point characters were clear and easily read.

B: Part of the images of 3 point character were unreadable but the images of 5 point character were easily read.

C: Almost all of the images of 3 point characters were unreadable and all or parts of the images of 5 point characters were also unreadable.

TABLE 2

| Photoreceptor No. | Potential variation at the solid black image area ( $\Delta V$ ) | Thinning of character image | Black spotting      | Recurring image defect | Cracking            | Image density       | Sharpness           | Remarks |
|-------------------|------------------------------------------------------------------|-----------------------------|---------------------|------------------------|---------------------|---------------------|---------------------|---------|
| 1A                | A                                                                | A                           | A                   | A                      | A                   | A                   | A                   | Inv.    |
| 2A                | A                                                                | A                           | A                   | A                      | A                   | A                   | A                   | Inv.    |
| 3A                | A                                                                | A                           | A                   | A                      | A                   | A                   | A                   | Inv.    |
| 4A                | A                                                                | A                           | A                   | A                      | A                   | A                   | A                   | Inv.    |
| 5A                | A                                                                | A                           | A                   | A                      | A                   | A                   | A                   | Inv.    |
| 6A                | A                                                                | A                           | A                   | A                      | A                   | A                   | A                   | Inv.    |
| 7A                | A                                                                | A                           | A                   | A                      | A                   | A                   | A                   | Inv.    |
| 8A                | A                                                                | A                           | A                   | A                      | A                   | A                   | A                   | Inv.    |
| 9A                | A                                                                | A                           | A                   | A                      | A                   | A                   | A                   | Inv.    |
| 10A               | A                                                                | A                           | A                   | A                      | A                   | A                   | A                   | Inv.    |
| 11A               | A                                                                | A                           | A                   | A                      | A                   | A                   | A                   | Inv.    |
| 12A               | B                                                                | B                           | A                   | B                      | B                   | B                   | B                   | Inv.    |
| 13A               | A                                                                | A                           | A                   | A                      | A                   | A                   | A                   | Inv.    |
| 14A               | A                                                                | B                           | B                   | A                      | B                   | B                   | B                   | Inv.    |
| 15A               | C                                                                | C                           | C                   | B                      | C                   | C                   | C                   | Comp.   |
| 16A               | Cannot be evaluated                                              | Cannot be evaluated         | Cannot be evaluated | Cannot be evaluated    | Cannot be evaluated | Cannot be evaluated | Cannot be evaluated | Comp.   |
| 17A               | C                                                                | B                           | B                   | C                      | C                   | C                   | C                   | Comp.   |

Inv.; Inventive

Comp.; Comparative

As is shown in Table 2, Photoreceptors 1A through 14A using the mixture of compounds as the charge transfer material in which  $(Rp+Rs)$  is not more than 99% are excellent in the high speed response, namely the potential variation of the solid black image area is small, under a low temperature and low humidity condition of 10°C. and 20% RH, accordingly thinning of the character image does not occur. In addition, the black spotting, the recurring image defects and the cracking are not observed with excellent image density and the sharpness. On the contrary, Photoreceptor 15A using only the low molecular weight compound of  $n=0$  is inferior in the high speed response under the low temperature and low humidity condition and causes the thinning of the character image. In addition, the layer is soft; the black spotting and the recurring image defects occur and the image density and the sharpness are also degraded. In the case of Photoreceptor 16A only using the high molecular weight compound of  $n=3$ , the compatibility of the compound with the binder resin is poor, and the photoreceptor has little sensitivity. Therefore, such a photoreceptor is not worth evaluation. In Photoreceptor 17A using a mixture of 50% of component  $n=1$  and 50% of component  $n=2$  of Compound 21A ( $p=0$ ,  $q=0$ ), solubility of the compound mixture with a binder resin is insufficient. Consequently, the potential variation of the solid black image portion is large and the recurring image defects and the cracking occur. In addition the image density and the sharpness are also lowered.

#### Example 2

Photoreceptors containing the mixture of compounds represented by Formula B were prepared as follows.

#### Preparation of Photoreceptor 1B

##### <Interlayer>

Polyamide resin, Amilan CM-8000 (Toray Co., Ltd.) 60 parts  
Inorganic particle: Titanium oxide SMT500SAS 180 parts

-continued

30 (Tayca Corporation, Surface treated by silica, alumina and methylhydrogenpolysiloxane)

Methanol 1600 parts  
1-butanol 400 parts

35 The above components were mixed and dissolved to prepare an interlayer coating liquid. The coating liquid was coated on a cylindrical aluminum substrate by the immersion coating method and dried to form a 1.0  $\mu\text{m}$  interlayer.

##### <Charge Generation Layer>

45 Titanylphthalocyanine (The highest peak of Bragg angle 20 at a 27.3° of Cu-K $\alpha$  characteristic X-ray diffraction) 60 parts  
Silicone resin solution, 15% xylene-butanol solution of 700 parts  
KR5240 (Shin'etsu Kagaku Co., Ltd.)  
2-butanol 2000 parts

50 The above components were mixed and dispersed by a sand mill for 10 hours to prepare a charge generation layer coating liquid. The coating liquid was applied onto the foregoing interlayer by an immersion method and dried. Thus a 0.3  $\mu\text{m}$  charge generation layer was formed.

##### <Charge Transfer Layer>

60 Charge transfer material, Compound of Synthesizing Example 4 150 parts  
Binder resin, bis-phenol Z type polycarbonate Eupiron Z 300 parts  
300 (Mitsubishi Gas Chemical Company Inc.)  
Antioxidant Sanol LS2626 (Sankyo Co., Ltd.) 1.7 parts  
Tetrahydrofuran (boiling point: 64.5 ° C.) 2200 parts

The above components were mixed and dissolved to prepare a charge transfer layer coating liquid. The coating liquid was applied onto the foregoing charge generation layer by an immersion coating method and dried for 40 minutes at 100° C. Thus a of 22  $\mu\text{m}$  charge transfer layer was formed to prepare Photoreceptor 1B.

#### Preparation of Photoreceptors 2B through 14B

Photoreceptors 2B through 14B were prepared in the same manner as Photoreceptor 1B except that the compound of charge generation material, the compound of charge transfer material and their amount and thickness of the charge transfer layer were changed as listed in Table 3.

#### Preparation of Photoreceptor 15B

Photoreceptor 15B was prepared in the same manner as Photoreceptor 1B except that the charge transfer material or the compound of Synthesizing Example 5 was replaced by the component n=0 of Compound 11B (m=0) synthesized by a commonly known method. The purity of the component was greater than 99%.

#### Preparation of Photoreceptor 16B

Photoreceptor 16B was prepared in the same manner as Photoreceptor 1B except that the charge transfer material or the compound of Synthesizing Example 5 was replaced by the component n=3 of Compound 11B (m=0) separated by liquid chromatography from the compound of Synthesizing Example 5. The purity of the component was larger than 99%. However, any photoreceptor capable of being evaluated could not be obtained since the compound was not compatible with the binder resin and precipitated.

#### Preparation of Photoreceptor 17B

Compound 11B (m=0) was separated by liquid chromatography into each component and a mixture of 50% of the component n=2 and 50% of n=3 was prepared. Then Photoreceptor 17B was prepared in the same manner as Photoreceptor 1B except that the charge transfer material was replaced by the above mixture.

TABLE 3

| Photo-<br>receptor<br>No. | Chemical<br>structure<br>*1 | No.<br>*2 | Charge transfer layer                                       |       |       |       |       |       |       |       |       |       |           |      | Average<br>molecular<br>weight |    |       |        | Re-<br>marks |  |  |
|---------------------------|-----------------------------|-----------|-------------------------------------------------------------|-------|-------|-------|-------|-------|-------|-------|-------|-------|-----------|------|--------------------------------|----|-------|--------|--------------|--|--|
|                           |                             |           | Charge transfer material (Compound and ratio of components) |       |       |       |       |       |       |       |       |       |           |      | (Rp + Rs)                      |    | (Mw)  | (Part) |              |  |  |
|                           |                             |           | m                                                           | n = 0 | n = 1 | n = 2 | n = 3 | n = 4 | n = 5 | n = 6 | n = 7 | n = 8 | (Rp + Rs) |      |                                |    |       |        |              |  |  |
| 1B                        | Y                           | 12B       | 0                                                           | 24.3  | 44.4  | 21.5  | 7.2   | 2.3   | 0.3   | 0.0   | 0.0   | 0.0   | 68.2      | 1542 | 150                            | 22 | Inv.  |        |              |  |  |
| 2B                        | Y                           | 11B       | 0                                                           | 32.5  | 45.0  | 16.0  | 5.3   | 1.2   | 0.0   | 0.0   | 0.0   | 0.0   | 77.5      | 1297 | 150                            | 22 | Inv.  |        |              |  |  |
| 3B                        | Y                           | 5B        | 0                                                           | 33.7  | 34.6  | 19.4  | 9.6   | 2.7   | 0.0   | 0.0   | 0.0   | 0.0   | 68.3      | 1653 | 150                            | 22 | Inv.  |        |              |  |  |
| 4B                        | Y                           | 12B       | 0                                                           | 24.3  | 44.4  | 21.5  | 7.2   | 2.3   | 0.3   | 0.0   | 0.0   | 0.0   | 68.7      | 1542 | 225                            | 27 | Inv.  |        |              |  |  |
| 5B                        | Y                           | 12B       | 0                                                           | 24.3  | 44.4  | 21.5  | 7.2   | 2.3   | 0.3   | 0.0   | 0.0   | 0.0   | 68.7      | 1542 | 100                            | 16 | Inv.  |        |              |  |  |
| 6B                        | Y                           | 15B       | 0                                                           | 22.1  | 43.8  | 21.0  | 9.8   | 3.0   | 0.3   | 0.0   | 0.0   | 0.0   | 65.9      | 1490 | 150                            | 22 | Inv.  |        |              |  |  |
| 7B                        | Y                           | 17B       | 0                                                           | 52.0  | 31.3  | 12.3  | 3.5   | 0.9   | 0.0   | 0.0   | 0.0   | 0.0   | 83.3      | 975  | 150                            | 22 | Inv.  |        |              |  |  |
| 8B                        | Z                           | 7B        | 1                                                           | 33.9  | 46.3  | 15.0  | 4.0   | 0.8   | 0.3   | 0.0   | 0.0   | 0.0   | 80.2      | 1663 | 150                            | 22 | Inv.  |        |              |  |  |
| 9B                        | Z                           | 13B       | 0                                                           | 25.4  | 40.8  | 18.1  | 6.3   | 1.4   | 0.0   | 0.0   | 0.0   | 0.0   | 76.2      | 1515 | 150                            | 22 | Inv.  |        |              |  |  |
| 10B                       | Y                           | 22B       | 0                                                           | 32.6  | 45.0  | 14.2  | 7.3   | 0.9   | 0.0   | 0.0   | 0.0   | 0.0   | 87.6      | 1784 | 150                            | 22 | Inv.  |        |              |  |  |
| 11B                       | Y                           | 20B       | 1                                                           | 19.8  | 36.1  | 28.6  | 10.4  | 4.1   | 1.0   | 0.0   | 0.0   | 0.0   | 64.7      | 1833 | 150                            | 22 | Inv.  |        |              |  |  |
| 12B                       | Y                           | 12B       | 0                                                           | 72.0  | 19.8  | 6.1   | 2.1   | 0.0   | 0.0   | 0.0   | 0.0   | 0.0   | 91.8      | 865  | 150                            | 22 | Inv.  |        |              |  |  |
| 13B                       | Y                           | 12B       | 0                                                           | 6.8   | 13.5  | 20.3  | 22.5  | 16.2  | 10.2  | 6.3   | 3.8   | 0.4   | 42.8      | 2259 | 150                            | 22 | Inv.  |        |              |  |  |
| 14B                       | Y                           | 12B       | 0                                                           | 15.2  | 24.2  | 31.2  | 18.2  | 8.1   | 2.3   | 0.8   | 0.0   | 0.0   | 55.4      | 1826 | 150                            | 22 | Inv.  |        |              |  |  |
| 15B                       | Y                           | 11B       | 0                                                           | 100   | 0.0   | 0.0   | 0.0   | 0.0   | 0.0   | 0.0   | 0.0   | 0.0   | 100       | 672  | 150                            | 22 | Comp. |        |              |  |  |
| 16B                       | Y                           | 11B       | 0                                                           | 0.0   | 0.0   | 0.0   | 100   | 0.0   | 0.0   | 0.0   | 0.0   | 0.0   | 100       | 1869 | 150                            | 22 | Comp. |        |              |  |  |
| 17B                       | Y                           | 11B       | 0                                                           | 0.0   | 0.0   | 50    | 50    | 0.0   | 0.0   | 0.0   | 0.0   | 0.0   | 100       | 1670 | 150                            | 22 | Comp. |        |              |  |  |

\*1; Charge generation layer

\*2; Charge generation material

Inv.; Inventive

Comp.; Comparative

In the above table, Y and Z are the same as those in Table 1.

(Rp+Rs) is the same as that in Table 1.

The distribution or the ratio of the n of the chain structure of the charge transfer material was determined from the area ratio of the high speed liquid chromatography. The average Mw was the weight average molecular weight in terms of polystyrene determined by the gel permeation chromatography.

#### Evaluation

Thus obtained Photoreceptors 1B through 17B were each installed into the reversal development digital copying machine Konica 7085 having a scorotron charging device, a semi-conductor laser exposing device emitting light at 680 nm and a reversal developing unit, and operated at a copying rate of 85 sheets of a4 size paper per minute, and evaluated in the same manner as Example 1. Results of the evaluation are listed in Table 4.

TABLE 4

| Photoreceptor No. | Potential variation at solid black image area ( $ \Delta V $ ) | Thinning of character image | Black spotting | Recurring image defect | Cracking | Image density | Sharpness | Remarks |
|-------------------|----------------------------------------------------------------|-----------------------------|----------------|------------------------|----------|---------------|-----------|---------|
| 1B                | A                                                              | A                           | A              | A                      | A        | A             | A         | Inv.    |
| 2B                | A                                                              | A                           | A              | A                      | A        | A             | A         | Inv.    |
| 3B                | A                                                              | A                           | A              | A                      | A        | A             | A         | Inv.    |
| 4B                | A                                                              | A                           | A              | A                      | A        | A             | A         | Inv.    |
| 5B                | A                                                              | A                           | A              | A                      | A        | A             | A         | Inv.    |
| 6B                | A                                                              | A                           | A              | A                      | A        | A             | A         | Inv.    |
| 7B                | A                                                              | A                           | A              | A                      | A        | A             | A         | Inv.    |
| 8B                | A                                                              | A                           | A              | A                      | A        | A             | A         | Inv.    |
| 9B                | A                                                              | A                           | A              | A                      | A        | A             | A         | Inv.    |
| 10B               | A                                                              | A                           | A              | A                      | A        | A             | A         | Inv.    |
| 11B               | A                                                              | A                           | A              | A                      | A        | A             | A         | Inv.    |
| 12B               | A                                                              | B                           | A              | B                      | A        | B             | B         | Inv.    |
| 13B               | B                                                              | B                           | A              | A                      | B        | B             | B         | Inv.    |
| 14B               | A                                                              | A                           | A              | A                      | A        | A             | A         | Inv.    |
| 15B               | C                                                              | C                           | C              | C                      | B        | C             | C         | Comp.   |
| 16B               | *1                                                             | *1                          | *1             | *1                     | *1       | *1            | *1        | Comp.   |
| 17B               | C                                                              | B                           | B              | C                      | C        | C             | C         | Comp.   |

Inv.; Inventive

Comp.; Comparative

\*1; Cannot be evaluated.

As is shown in Table 4, Photoreceptors 1B through 14B using the mixture of compounds as the charge transfer material in each of which (Rp+Rs) is not more than 99% are excellent in the high speed response, namely the potential variation of the solid black image area is small, under low temperature and humidity conditions of 10°C. and 20% RH, so that thinning of image characters does not occur. In addition, the black spotting, the recurring image defects and the cracking are not formed and excellent in the image density and the sharpness. Contrary, Photoreceptor 15B only using the low molecular weight n=0 compound is inferior in the high speed response under the low temperature and humidity condition and causes the thinning of the character image. In addition, the layer is soft; black spotting and recurring image defects occur, and in addition image density and sharpness are also degraded. In the case of Photorecep-

tor 16B using only the high molecular weight compound n=3, the compatibility of the compound with the binder resin is poor, and the photoreceptor has little sensitivity. Therefore, such a photoreceptor is not worth evaluation. In Photoreceptor 17B using the mixture of 50% of component n=2 and 50% of component n=3 of Compound 11B (m=0), the solubility of the compound mixture with the binder resin is insufficient. Consequently, the potential variation at solid black image area is wide and the recurring image defects and the cracking occur. In addition image density and sharpness are also lowered.

#### Example 3

Photoreceptors containing the mixture of compounds represented by Formula C were prepared as follows.

15

#### Preparation of Photoreceptor 1C

##### <Interlayer>

|    |                                                                                        |            |
|----|----------------------------------------------------------------------------------------|------------|
| 55 | Polyamide resin, Amilan CM-8000 (Toray Co., Ltd.)                                      | 60 parts   |
|    | Inorganic particle: Titanium oxide SMT500SAS                                           | 180 parts  |
|    | (Tayca Corporation, Surface treated by silica, alumina and methylhydrogenpolysiloxane) |            |
| 60 | Methanol                                                                               | 1600 parts |
|    | 1-butanol                                                                              | 400 parts  |

The above components were mixed and dissolved to prepare an interlayer coating liquid. The coating liquid was coated on a cylindrical aluminum substrate by an immersion coating method and dried to form a 1.0 μm interlayer.

## &lt;Charge Generation Layer&gt;

|                                                                                                                          |            |
|--------------------------------------------------------------------------------------------------------------------------|------------|
| Titanylphthalocyanine (The highest peak of a Bragg angle 20 at 27.3° for Cu-K $\alpha$ characteristic X-ray diffraction) | 60 parts   |
| Silicone resin solution, 15% xylene-butanol solution of KR5240 (Shin'etsu Kagaku Co., Ltd.)                              | 700 parts  |
| 2-butanone                                                                                                               | 2000 parts |

The above components were mixed and dispersed by a sand mill for 10 hours to prepare a charge generation layer coating liquid. The coating liquid is coated onto the foregoing interlayer by the immersion method and dried. Thus a 0.3  $\mu$ m charge generation layer was formed.

## &lt;Charge Transfer Layer&gt;

|                                                                                           |            |
|-------------------------------------------------------------------------------------------|------------|
| Charge transfer material, Compound of Synthesizing Example 4                              | 150 parts  |
| Binder resin, bis-phenol Z type polycarbonate Eupiron Z 300 (Mitsubishi Kagaku Co., Ltd.) | 300 parts  |
| Antioxidant Sanol LS2626 (Sankyo Co., Ltd.)                                               | 1.7 parts  |
| Tetrahydrofuran (boiling point: 64.5° C.)                                                 | 2200 parts |

The above components were mixed and dissolved to prepare a charge transfer layer coating liquid. The coating liquid was coated on the foregoing charge generation by the immersion coating method and dried for 40 minutes at 100° C. Thus a charge transfer layer with a thickness of 22  $\mu$ m was formed to prepare Photoreceptor 1C.

## Preparation of Photoreceptor 2C

Photoreceptor 2C was prepared in the same manner as Photoreceptor 1C except that the compound of Synthesizing Example 6 was replaced by the compound of Synthesizing Example 7.

## Preparation of Photoreceptors 3C through 10C

Photoreceptors 3C through 10C were prepared in the same manner as Photoreceptor 1C except that the compound of charge generation material, the compound of charge transfer material and the amount of them and the thickness of the charge transfer layer were changed as listed in table 5.

## Preparation of Photoreceptor 11C

Photoreceptor 11C was prepared in the same manner as Photoreceptor 1C except that the charge transfer material or the compound of Synthesizing Example 6 was replaced by the component n=0 of Compound 17C synthesized by the known method. The purity of the component was larger than 99%.

## Preparation of Photoreceptor 12C

Photoreceptor 12C was prepared in the same manner as Photoreceptor 1C except that the charge transfer material or the compound of Synthesizing Example 6 was replaced by the component n=4 of Chemical Structure 17C separated by liquid chromatography from the compound of Synthesizing Example 6. The purity of the component was larger than 99%. However, any photoreceptor capable of being subjected to the evaluation cannot be obtained since the compound was not permissible with the binder resin and precipitated.

## Preparation of Photoreceptor 13C

The compound of Synthesizing Example 6 was separated by liquid chromatography into each component and a mixture of 50% of the component n=3 and 50% of that of n=4 of Chemical Structure was prepared. Then Photoreceptor 13C was prepared in the same manner as Photoreceptor 1C except that the charge transfer material was replaced by the above mixture.

TABLE 5

| *1  | *2 | *3  | *4 | Charge transfer layer |       |       |       |       |       |       |       |       |       |        |        | (Rp + Rs) | Average molecular weight (Mw) | Amount (Part) | Re-*5 marks |
|-----|----|-----|----|-----------------------|-------|-------|-------|-------|-------|-------|-------|-------|-------|--------|--------|-----------|-------------------------------|---------------|-------------|
|     |    |     |    | n = 0                 | n = 1 | n = 2 | n = 3 | n = 4 | n = 5 | n = 6 | n = 7 | n = 8 | n = 9 | n = 10 | n = 11 |           |                               |               |             |
| 1C  | Y  | 17C |    | 14.8                  | 25.1  | 27.4  | 18.1  | 9.9   | 3.4   | 1.1   | 0.2   | 0.0   | 0.0   | 0.0    | 0.0    | 52.5      | 910                           | 150           | 22 Inv.     |
| 2C  | Y  | 48C |    | 0.9                   | 3.4   | 12.0  | 22.8  | 31.3  | 19.9  | 6.9   | 2.5   | 0.3   | 0.0   | 0.0    | 0.0    | 54.1      | 1684                          | 150           | 22 Inv.     |
| 3C  | Y  | 53C |    | 7.4                   | 14.5  | 19.3  | 20.0  | 17.1  | 11.5  | 6.1   | 3.2   | 0.9   | 0.0   | 0.0    | 0.0    | 39.3      | 1680                          | 150           | 22 Inv.     |
| 4C  | Y  | 17C |    | 23.5                  | 40.1  | 21.5  | 10.4  | 3.8   | 0.7   | 0.0   | 0.0   | 0.0   | 0.0   | 0.0    | 0.0    | 63.6      | 660                           | 150           | 22 Inv.     |
| 5C  | Y  | 17C |    | 32.1                  | 47.0  | 15.4  | 4.4   | 1.1   | 0.0   | 0.0   | 0.0   | 0.0   | 0.0   | 0.0    | 0.0    | 79.1      | 523                           | 225           | 27 Inv.     |
| 6C  | Y  | 17C |    | 0.6                   | 2.5   | 7.0   | 10.5  | 14.1  | 16.3  | 16.2  | 13.1  | 0.1   | 6.7   | 2.5    | 0.5    | 32.5      | 1520                          | 150           | 16 Inv.     |
| 7C  | Z  | 17C |    | 14.8                  | 25.1  | 27.4  | 18.1  | 9.9   | 3.4   | 1.1   | 0.2   | 0.0   | 0.0   | 0.0    | 0.0    | 52.5      | 910                           | 150           | 22 Inv.     |
| 8C  | Z  | 48C |    | 0.9                   | 3.4   | 12.0  | 22.8  | 31.3  | 19.9  | 6.9   | 2.5   | 0.3   | 0.0   | 0.0    | 0.0    | 54.1      | 1684                          | 150           | 22 Inv.     |
| 9C  | Y  | 38C |    | 6.9                   | 13.8  | 20.2  | 21.1  | 17.1  | 11.0  | 5.9   | 2.7   | 1.3   | 0.0   | 0.0    | 0.0    | 41.3      | 1186                          | 150           | 22 Inv.     |
| 10C | Y  | 17C |    | 62.9                  | 28.1  | 6.2   | 1.8   | 0.0   | 0.0   | 0.0   | 0.0   | 0.0   | 0.0   | 0.0    | 0.0    | 91.0      | 471                           | 150           | 22 Inv.     |
| 11C | Y  | 17C |    | 0.0                   | 100   | 0.0   | 0.0   | 0.0   | 0.0   | 0.0   | 0.0   | 0.0   | 0.0   | 0.0    | 0.0    | 100       | 468                           | 150           | 22 Comp.    |
| 12C | Y  | 17C |    | 0.0                   | 0.0   | 0.0   | 0.0   | 100   | 0.0   | 0.0   | 0.0   | 0.0   | 0.0   | 0.0    | 0.0    | 100       | 1053                          | 150           | 22 Comp.    |
| 13C | Y  | 17C |    | 0.0                   | 0.0   | 0.0   | 50    | 50    | 0.0   | 0.0   | 0.0   | 0.0   | 0.0   | 0.0    | 0.0    | 100       | 956                           | 150           | 22 Comp.    |

\*1; Photoreceptor No.

\*2; Charge generation layer

\*3; Charge generation material

\*4; Chemical structure No.

\*5; Layer thickness ( $\mu$ m)

Inv.; Inventive

Comp.; Comparative

In the above table, Y and Z are the same as those in Table 1.

(Rp+Rs) is the same as that in Table 1.

The distribution or the ratio of the n of the chain structure of the charge transfer material was determined from the area ratio via high speed liquid chromatography GPC. The average Mw was the weight average molecular weight converted to polystyrene determined by gel permeation chromatography.

#### Evaluation

Thus obtained Photoreceptors 1C through 13C were each installed into a being a reversal development digital copying machine Konica 7085 having a scorotron charging device, a semi-conductor laser exposing device emitting light at 680 nm and a reversal developing unit, and operation of a copying rate of 85 sheets of A4 size paper per minute, and was evaluated in the same manner as in Example 1. Results of the evaluation are shown in Table 6.

TABLE 6

| Photoreceptor No. | Potential variation at solid black image area ( $ \Delta V $ ) | Thinning of character image | Black spotting       | Recurring image defect | Cracking             | Image density        | Sharpness            | Remarks |
|-------------------|----------------------------------------------------------------|-----------------------------|----------------------|------------------------|----------------------|----------------------|----------------------|---------|
| 1C                | A                                                              | A                           | A                    | A                      | A                    | A                    | A                    | Inv.    |
| 2C                | A                                                              | A                           | A                    | A                      | A                    | A                    | A                    | Inv.    |
| 3C                | A                                                              | A                           | A                    | A                      | A                    | A                    | A                    | Inv.    |
| 4C                | A                                                              | A                           | A                    | A                      | A                    | A                    | A                    | Inv.    |
| 5C                | A                                                              | A                           | A                    | A                      | A                    | A                    | A                    | Inv.    |
| 6C                | B                                                              | B                           | B                    | B                      | A                    | B                    | B                    | Inv.    |
| 7C                | A                                                              | A                           | A                    | A                      | A                    | A                    | A                    | Inv.    |
| 8C                | A                                                              | A                           | A                    | A                      | A                    | A                    | A                    | Inv.    |
| 9C                | B                                                              | B                           | A                    | A                      | B                    | B                    | B                    | Inv.    |
| 10C               | A                                                              | B                           | A                    | B                      | A                    | B                    | B                    | Inv.    |
| 11C               | C                                                              | C                           | C                    | B                      | C                    | C                    | C                    | Comp.   |
| 12C               | Cannot be evaluated.                                           | Cannot be evaluated.        | Cannot be evaluated. | Cannot be evaluated.   | Cannot be evaluated. | Cannot be evaluated. | Cannot be evaluated. | Comp.   |
| 13C               | C                                                              | B                           | B                    | C                      | C                    | C                    | C                    | Comp.   |

Inv.; Inventive  
Comp.; Comparative

As is shown in Table 6, Photoreceptors 1C through 10C using the mixture of compounds as the charge transfer material in each of which (Rp+Rs) is not more than 99% are excellent in the high speed response, namely the potential variation of the solid black image area is small, under low temperature and low humidity condition of 10° C. and 20% RH, accordingly thinning of the character image does not occur. In addition, the black spotting, the recurring image defect and the cracking are not formed and results in excellent image density and sharpness. On the contrary, Photoreceptor 11C using only the low molecular weight compound n=1 is inferior in the high speed response under low temperature and humidity condition and causes thinning of image characters. In addition, the layer is soft; black spotting and recurring image defects occur and image density and sharpness are also degraded. In the case of Photoreceptor 12C using only the high molecular weight compound n=4, the compatibility of the compound with a binder resin is poor, and the photoreceptor exhibits low sensitivity. Therefore, such a photoreceptor is not worth evaluation. In Photoreceptor 13C using the mixture of 50% of component n=3 and 50% of component n=4 of Chemical Structure 17C, the solubility of the compound mixture with the binder resin is insufficient. Consequently, the potential variation at the

solid black image area is wide and recurring image defects and cracking occur. In addition the image density and the sharpness are also lowered.

5 The invention claimed is:

1. An electrophotographic photoreceptor comprising a support and a photosensitive layer, wherein the photosensitive layer contains a mixture of two or more compounds each of which is represented by Formula (1) having a specific number n different each other,



wherein CTM-group is a charge transfer group; X and Y are each a hydrogen atom, a halogen atom or a mono-15 valent organic group; and n is an integer of 0 to 10, provided that n is not 0 when both X and Y are a hydrogen atom or a halogen atom, and (Rp+Rs) is not more than 99%,

15

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

97

7. The electrophotographic photoreceptor of claim 1, wherein the CTM-group, X and Y in Formula (1) are each represented by following formula, respectively,

CTM-group



wherein Ar<sub>1</sub> is a substituted or unsubstituted mono-valent aromatic group; Ar<sub>2</sub> is a di-valent substituted or unsubstituted aromatic group, a di-valent furan or thiophene group; or a group represented by Formula (2); R<sub>1</sub> through R<sub>3</sub> are each a hydrogen atom, a substituted or unsubstituted alkyl group or a substituted or unsubstituted mono-valent aromatic group; A is a di-valent group having a triaryl amino group or a group represented by Formula (3), plural Ar<sub>1</sub>, R<sub>1</sub>, R<sub>2</sub> and R<sub>3</sub> may be the same or different from each other, and p and q are each an integer of 0 or 1,



Formula (2)

wherein Z is a single bond, an oxygen atom, a sulfur atom, a —CH=CH— group or a —C(R<sub>4</sub>)(R<sub>5</sub>)— group, and R<sub>4</sub> and R<sub>5</sub> may bond with together,



Formula (3)

wherein Z<sub>1</sub> is a single bond, an alkylene group, an oxygen atom or a sulfur atom; and R<sub>sub.6</sub> is a substituted or unsubstituted alkyl group, or substituted or unsubstituted aromatic group.

8. The electrophotographic photoreceptor of claim 7, wherein the divalent group having the triaryl amino group is a group represented by the following Formula (4),



Formula (4)

98

wherein Ar<sub>3</sub> is a substituted or unsubstituted mono-valent aromatic group.

9. The electrophotographic photoreceptor of claim 7, wherein the group represented by Ar<sub>3</sub> is a group represented by Formula (5),



Formula (5)

wherein R<sub>31</sub>, R<sub>32</sub>, R<sub>33</sub>, R<sub>34</sub> and R<sub>35</sub> are each a hydrogen atom or an alkyl group having from 1 to 4 carbon atoms and at least one of R<sub>31</sub> and R<sub>35</sub> is an alkyl group having from 1 to 4 carbon atoms.

10. The electrophotographic photoreceptor of claim 7, wherein the di-valent group having a triaryl amino group is a group represented by Formula (6),



Formula (6)

wherein X<sub>2</sub> is a single bond, a substituted or unsubstituted alkylene group, or a substituted or unsubstituted di-valent aromatic group; Ar<sub>4</sub> and Ar<sub>5</sub> are each a substituted or unsubstituted mono-valent aromatic group.

11. The electrophotographic photoreceptor of claim 1, wherein CTM-group, X and Y in Formula (1) are each represented by the following formula, respectively,

CTM-group



wherein, Ar<sub>2</sub> is a substituted or unsubstituted di-valent aromatic group, a di-valent furan or thiophene group or a group represented by Formula (2); R<sub>1</sub> through R<sub>3</sub> are each a hydrogen atom, a substituted or unsubstituted alkyl group, or a substituted or unsubstituted mono-valent aromatic group; A is a divalent group having a triaryl amino group or a group represented by Formula (3); and Ar<sub>1</sub> is a substituted or unsubstituted mono-valent aromatic group; plural Ar<sub>1</sub>, R<sub>1</sub>, R<sub>2</sub> and R<sub>3</sub> each may be the same or different from each other and m is an integer of 0 or 1.

12. The electrophotographic photoreceptor of claim 11, wherein the divalent group having the triaryl amino group is a group represented by the following Formula (4),

99



wherein Ar<sub>3</sub> is a substituted or unsubstituted mono-valent aromatic group.

13. The electrophotographic photoreceptor of claim 11, wherein the group represented by Ar<sub>3</sub> is a group represented by Formula (5),



wherein R<sub>31</sub>, R<sub>32</sub>, R<sub>33</sub>, R<sub>34</sub> and R<sub>35</sub> are each a hydrogen atom or an alkyl group having from 1 to 4 carbon atoms and at least one of R<sub>31</sub> and R<sub>35</sub> is an alkyl group having from 1 to 4 carbon atoms.

14. The electrophotographic photoreceptor of claim 11, wherein the di-valent group having a triarylamino group is a group represented by Formula (6),



wherein X<sub>2</sub> is a single bond, a substituted or unsubstituted alkylene group, or a substituted or unsubstituted di-valent aromatic group; Ar<sub>4</sub> and Ar<sub>5</sub> are each a substituted or unsubstituted mono-valent aromatic group.

15. The electrophotographic photoreceptor of claim 11, wherein Ar<sub>1</sub> is a group represented by Formula (7)



Formula (4)

5

100

wherein R<sub>41</sub>, R<sub>42</sub>, R<sub>43</sub>, R<sub>44</sub>, R<sub>45</sub>, R<sub>51</sub>, R<sub>52</sub>, R<sub>53</sub>, R<sub>54</sub> and R<sub>55</sub> are each a hydrogen atom or an alkyl group having from 1 to 4 carbon atoms, provided that at least one of R<sub>41</sub>, R<sub>45</sub>, R<sub>51</sub> and R<sub>55</sub> is an alkyl group having from 1 to 4 carbon atoms.

16. The electrophotographic photoreceptor of claim 1, wherein the CTM-group in Formula (1), X, and Y are each represented by Formula C



wherein Ar<sub>1</sub> is a substituted or unsubstituted mono-valent aromatic group; Ar<sub>6</sub> is a substituted or unsubstituted di-valent aromatic group, or a group represented by the following Formula (8); R is a substituted or unsubstituted alkyl group or a substituted or unsubstituted mono-valent aromatic group, and plural Ar<sub>1</sub>, Ar<sub>6</sub> and R may be the same or different from each other,



wherein Z<sub>3</sub> is an oxygen atom, a sulfur atom, a —CH=CH— group or a —CH<sub>2</sub>—CH<sub>2</sub>— group; and R<sub>81</sub> and R<sub>82</sub> are each a hydrogen atom or an alkyl group having from 1 to 4 carbon atoms.

17. A processing cartridge comprising the electrophotographic photoreceptor of claim 1, and at least one of a charging unit for uniformly charging the surface of the electrophotographic photoreceptor, a latent image forming unit for forming a latent image on the charged electrophotographic photoreceptor, a developing unit for visualizing the latent image formed on the electrophotographic photoreceptor, a transferring unit for transferring the toner image visualized on the electrophotographic photoreceptor to a recording material, a discharging unit for removing the charge on the electrophotographic photoreceptor and a cleaning unit for removing the toner remaining on the electrophotographic photoreceptor, and is installed and released to from a main body of an image forming apparatus.

\* \* \* \* \*